



US010016810B2

(12) **United States Patent**  
**Salinas et al.**

(10) **Patent No.:** **US 10,016,810 B2**  
(b5) **Date of Patent:** **Jul. 10, 2018**

(54) **METHODS OF MANUFACTURING  
DEGRADABLE TOOLS USING A GALVANIC  
CARRIER AND TOOLS MANUFACTURED  
THEREOF**

(71) Applicants: **Bobby J. Salinas**, Houston, TX (US);  
**Zhiyue Xu**, Cypress, TX (US)

(72) Inventors: **Bobby J. Salinas**, Houston, TX (US);  
**Zhiyue Xu**, Cypress, TX (US)

(73) Assignee: **BAKER HUGHES, A GE  
COMPANY, LLC**, Houston, TX (US)

(\*) Notice: Subject to any disclaimer, the term of this  
patent is extended or adjusted under 35  
U.S.C. 154(b) by 302 days.

(21) Appl. No.: **14/967,420**

(22) Filed: **Dec. 14, 2015**

(65) **Prior Publication Data**

US 2017/0165745 A1 Jun. 15, 2017

(51) **Int. Cl.**

**B22D 18/06** (2006.01)  
**B22D 23/06** (2006.01)  
**E21B 33/12** (2006.01)

(52) **U.S. Cl.**

CPC ..... **B22D 18/06** (2013.01); **B22D 23/06**  
(2013.01); **E21B 33/12** (2013.01)

(58) **Field of Classification Search**

CPC ..... B22D 18/06; B22D 23/06; E21B 33/12

USPC ..... 428/404

See application file for complete search history.

(56) **References Cited**

U.S. PATENT DOCUMENTS

1,468,905 A 9/1923 Herman  
1,558,066 A 10/1925 Veazey et al.  
2,189,697 A 2/1940 Baker  
2,222,233 A 11/1940 Mize  
2,225,143 A 12/1940 Baker et al.  
2,238,895 A 4/1941 Gage  
2,261,292 A 11/1941 Salnikov  
2,294,648 A 9/1942 Ansel  
2,301,624 A 11/1942 Holt  
2,352,993 A 7/1944 Albertson  
2,394,843 A 2/1946 Cooke et al.  
2,672,199 A 3/1954 McKenna  
2,753,941 A 7/1956 Hebard et al.  
2,754,910 A 7/1956 Derrick et al.  
2,933,136 A 4/1960 Ayers et al.  
2,983,634 A 5/1961 Budininkas et al.  
3,057,405 A 10/1962 Mallinger  
3,066,391 A 12/1962 Vordahl  
3,106,959 A 10/1963 Huitt et al.  
3,142,338 A 7/1964 Brown  
3,152,009 A 10/1964 Delong  
3,180,728 A 4/1965 Keir et al.  
3,196,949 A 7/1965 Thomas  
3,226,314 A 12/1965 Wellington et al.  
3,242,988 A 3/1966 McGuire et al.  
3,316,748 A 5/1967 Lang et al.  
3,326,291 A 6/1967 Zandmer et al.

3,343,537 A 9/1967 Graham  
3,347,317 A 10/1967 Zandmer  
3,347,714 A 10/1967 Broverman et al.  
3,390,724 A 7/1968 Caldwell  
3,395,758 A 8/1968 Kelly et al.  
3,406,101 A 10/1968 Kilpatrick  
3,416,918 A 12/1968 Roberts  
3,465,181 A 9/1969 Colby et al.  
3,489,218 A 1/1970 Means  
3,513,230 A 5/1970 Rhee et al.  
3,600,163 A 8/1971 Badia et al.  
3,602,305 A 8/1971 Kisling  
3,637,446 A 1/1972 Elliott et al.  
3,645,331 A 2/1972 Maurer et al.  
3,660,049 A 5/1972 Benjamin  
3,765,484 A 10/1973 Hamby, Jr. et al.  
3,768,563 A 10/1973 Blount  
3,775,823 A 12/1973 Adolph et al.  
3,816,080 A 6/1974 Bomford et al.  
3,878,889 A 4/1975 Seabourn  
3,894,850 A 7/1975 Kovalchuk et al.  
3,924,677 A 12/1975 Prenner et al.  
3,957,483 A 5/1976 Suzuki  
4,010,583 A 3/1977 Highberg  
4,039,717 A 8/1977 Titus  
4,050,529 A 9/1977 Tagirov et al.  
4,157,732 A 6/1979 Fonner  
4,248,307 A 2/1981 Silberman et al.  
4,284,137 A 8/1981 Taylor  
4,292,377 A 9/1981 Petersen et al.  
4,372,384 A 2/1983 Kinney  
4,373,584 A 2/1983 Silberman et al.  
4,373,952 A 2/1983 Parent  
4,374,543 A 2/1983 Richardson  
4,384,616 A 5/1983 Dellingar  
4,395,440 A 7/1983 Abe et al.  
4,399,871 A 8/1983 Adkins et al.  
4,407,368 A 10/1983 Erbstoesser  
4,422,508 A 12/1983 Rutledge, Jr. et al.

(Continued)

FOREIGN PATENT DOCUMENTS

CA 2783241 A1 6/2011  
CA 2783346 A1 6/2011

(Continued)

OTHER PUBLICATIONS

"Declaration of Karl T. Hartwig in Support of Petitioner Pursuant to 37 C.F.R. § 42.120", executed on Nov. 21, 2016 in support of U.S. Pat. No. 8,573,295, 52 pages.

(Continued)

*Primary Examiner* — Leszek Kiliman

(74) *Attorney, Agent, or Firm* — Cantor Colburn LLP

(57) **ABSTRACT**

A method of manufacturing a degradable article comprises: forming a mixture comprising composite particles dispersed in a metallic matrix material; the composite particles comprising a carrier and a disintegration agent coated on the carrier or embedded in the carrier, or a combination thereof and having a density that is about 0.2 to about 2.5 equivalents to that of the metallic matrix material when measured under the same testing conditions; and molding or casting the mixture to form a degradable article. The disintegration agent forms a plurality of galvanic cells with the metallic matrix material, or the carrier, or a combination thereof, in the degradable article.

# US 10,016,810 B2

Page 2

---

| (56)                  | References Cited |                       |             |          |                          |
|-----------------------|------------------|-----------------------|-------------|----------|--------------------------|
| U.S. PATENT DOCUMENTS |                  |                       |             |          |                          |
|                       |                  |                       |             |          |                          |
| 4,450,136 A           | 5/1984           | Dudek et al.          | 5,103,911 A | 4/1992   | Heijnen                  |
| 4,452,311 A           | 6/1984           | Speegle et al.        | 5,117,915 A | 6/1992   | Mueller et al.           |
| 4,475,729 A           | 10/1984          | Costigan              | 5,161,614 A | 11/1992  | Wu et al.                |
| 4,498,543 A           | 2/1985           | Pye et al.            | 5,171,734 A | 12/1992  | Sanjurjo et al.          |
| 4,499,048 A           | 2/1985           | Hanejko               | 5,178,216 A | 1/1993   | Giroux et al.            |
| 4,499,049 A           | 2/1985           | Hanejko               | 5,181,571 A | 1/1993   | Mueller et al.           |
| 4,524,825 A           | 6/1985           | Fore                  | 5,183,631 A | 2/1993   | Kugimiya et al.          |
| 4,526,840 A           | 7/1985           | Jerabek               | 5,188,182 A | 2/1993   | Echols, III et al.       |
| 4,534,414 A           | 8/1985           | Pringle               | 5,188,183 A | 2/1993   | Hopmann et al.           |
| 4,539,175 A           | 9/1985           | Lichti et al.         | 5,204,055 A | 4/1993   | Sachs et al.             |
| 4,554,986 A           | 11/1985          | Jones                 | 5,222,867 A | 6/1993   | Walker, Sr. et al.       |
| 4,619,699 A           | 10/1986          | Petkovic-Luton et al. | 5,226,483 A | 7/1993   | Williamson, Jr.          |
| 4,640,354 A           | 2/1987           | Boisson               | 5,228,518 A | 7/1993   | Wilson et al.            |
| 4,648,901 A           | 3/1987           | Murray et al.         | 5,234,055 A | 8/1993   | Cornette                 |
| 4,664,962 A           | 5/1987           | Desmarais, Jr.        | 5,240,742 A | * 8/1993 | Johnson ..... B22F 1/025 |
| 4,668,470 A           | 5/1987           | Gilman et al.         |             |          | 427/216                  |
| 4,674,572 A           | 6/1987           | Gallus                | 5,252,365 A | 10/1993  | White                    |
| 4,678,037 A           | 7/1987           | Smith                 | 5,253,714 A | 10/1993  | Davis et al.             |
| 4,681,133 A           | 7/1987           | Weston                | 5,271,468 A | 12/1993  | Streich et al.           |
| 4,688,641 A           | 8/1987           | Knieriem              | 5,273,569 A | 12/1993  | Gilman et al.            |
| 4,690,796 A           | 9/1987           | Paliwal               | 5,282,509 A | 2/1994   | Schurr, III              |
| 4,693,863 A           | 9/1987           | Del Corso et al.      | 5,292,478 A | 3/1994   | Scorey                   |
| 4,703,807 A           | 11/1987          | Weston                | 5,293,940 A | 3/1994   | Hromas et al.            |
| 4,706,753 A           | 11/1987          | Ohkochi et al.        | 5,304,260 A | 4/1994   | Aikawa et al.            |
| 4,708,202 A           | 11/1987          | Sukup et al.          | 5,304,588 A | 4/1994   | Boysen et al.            |
| 4,708,208 A           | 11/1987          | Halbardier            | 5,309,874 A | 5/1994   | Willermet et al.         |
| 4,709,761 A           | 12/1987          | Setterberg, Jr.       | 5,310,000 A | 5/1994   | Arterbury et al.         |
| 4,714,116 A           | 12/1987          | Brunner               | 5,316,598 A | 5/1994   | Chang et al.             |
| 4,716,964 A           | 1/1988           | Erbstoesser et al.    | 5,318,746 A | 6/1994   | Lashmore                 |
| 4,719,971 A           | 1/1988           | Owens                 | 5,352,522 A | 10/1994  | Kugimiya et al.          |
| 4,721,159 A           | 1/1988           | Ohkochi et al.        | 5,380,473 A | 1/1995   | Bogue et al.             |
| 4,738,599 A           | 4/1988           | Shilling              | 5,387,380 A | 2/1995   | Cima et al.              |
| 4,741,973 A           | 5/1988           | Condit et al.         | 5,392,860 A | 2/1995   | Ross                     |
| 4,768,588 A           | 9/1988           | Kupsa                 | 5,394,236 A | 2/1995   | Murnick                  |
| 4,775,598 A           | 10/1988          | Jaekel                | 5,394,941 A | 3/1995   | Venditto et al.          |
| 4,784,226 A           | 11/1988          | Wyatt                 | 5,398,754 A | 3/1995   | Dinhoble                 |
| 4,805,699 A           | 2/1989           | Halbardier            | 5,407,011 A | 4/1995   | Layout                   |
| 4,817,725 A           | 4/1989           | Jenkins               | 5,409,555 A | 4/1995   | Fujita et al.            |
| 4,834,184 A           | 5/1989           | Streich et al.        | 5,411,082 A | 5/1995   | Kennedy                  |
| H635 H                | 6/1989           | Johnson et al.        | 5,417,285 A | 5/1995   | Van Buskirk et al.       |
| 4,850,432 A           | 7/1989           | Porter et al.         | 5,425,424 A | 6/1995   | Reinhardt et al.         |
| 4,853,056 A           | 8/1989           | Hoffman               | 5,427,177 A | 6/1995   | Jordan, Jr. et al.       |
| 4,869,324 A           | 9/1989           | Holder                | 5,435,392 A | 7/1995   | Kennedy                  |
| 4,869,325 A           | 9/1989           | Halbardier            | 5,439,051 A | 8/1995   | Kennedy et al.           |
| 4,880,059 A           | 11/1989          | Brandell et al.       | 5,454,430 A | 10/1995  | Kennedy et al.           |
| 4,889,187 A           | 12/1989          | Terrell et al.        | 5,456,317 A | 10/1995  | Hood, III et al.         |
| 4,890,675 A           | 1/1990           | Dew                   | 5,456,327 A | 10/1995  | Denton et al.            |
| 4,901,794 A           | 2/1990           | Baugh et al.          | 5,464,062 A | 11/1995  | Blizzard, Jr.            |
| 4,909,320 A           | 3/1990           | Hebert et al.         | 5,472,048 A | 12/1995  | Kennedy et al.           |
| 4,921,664 A           | 5/1990           | Couper                | 5,474,131 A | 12/1995  | Jordan, Jr. et al.       |
| 4,929,415 A           | 5/1990           | Okazaki               | 5,477,923 A | 12/1995  | Jordan, Jr. et al.       |
| 4,932,474 A           | 6/1990           | Schroeder, Jr. et al. | 5,479,986 A | 1/1996   | Gano et al.              |
| 4,938,309 A           | 7/1990           | Emdy                  | 5,506,055 A | 4/1996   | Dorfman et al.           |
| 4,944,351 A           | 7/1990           | Eriksen et al.        | 5,507,439 A | 4/1996   | Story                    |
| 4,949,788 A           | 8/1990           | Szarka et al.         | 5,511,620 A | 4/1996   | Baugh et al.             |
| 4,952,902 A           | 8/1990           | Kawaguchi et al.      | 5,524,699 A | 6/1996   | Cook                     |
| 4,975,412 A           | 12/1990          | Okazaki et al.        | 5,526,880 A | 6/1996   | Jordan, Jr. et al.       |
| 4,977,958 A           | 12/1990          | Miller                | 5,526,881 A | 6/1996   | Martin et al.            |
| 4,981,177 A           | 1/1991           | Carmody et al.        | 5,529,746 A | 6/1996   | Knoss et al.             |
| 4,986,361 A           | 1/1991           | Mueller et al.        | 5,533,573 A | 7/1996   | Jordan, Jr. et al.       |
| 4,997,622 A           | 3/1991           | Regazzoni et al.      | 5,536,485 A | 7/1996   | Kume et al.              |
| 5,006,044 A           | 4/1991           | Walker, Sr. et al.    | 5,558,153 A | 9/1996   | Holcombe et al.          |
| 5,010,955 A           | 4/1991           | Springer              | 5,601,924 A | 2/1997   | Beane                    |
| 5,036,921 A           | 8/1991           | Pittard et al.        | 5,607,017 A | 3/1997   | Owens et al.             |
| 5,048,611 A           | 9/1991           | Cochran               | 5,623,993 A | 4/1997   | Van Buskirk et al.       |
| 5,049,165 A           | 9/1991           | Tselenis              | 5,623,994 A | 4/1997   | Robinson                 |
| 5,061,323 A           | 10/1991          | Deluccia              | 5,636,691 A | 6/1997   | Hendrickson et al.       |
| 5,063,775 A           | 11/1991          | Walker, Sr. et al.    | 5,641,023 A | 6/1997   | Ross et al.              |
| 5,073,207 A           | 12/1991          | Faure et al.          | 5,647,444 A | 7/1997   | Williams                 |
| 5,074,361 A           | 12/1991          | Brisco et al.         | 5,665,289 A | 9/1997   | Chung et al.             |
| 5,076,869 A           | 12/1991          | Bourell et al.        | 5,677,372 A | 10/1997  | Yamamoto et al.          |
| 5,084,088 A           | 1/1992           | Okazaki               | 5,685,372 A | 11/1997  | Gano                     |
| 5,087,304 A           | 2/1992           | Chang et al.          | 5,701,576 A | 12/1997  | Fujita et al.            |
| 5,090,480 A           | 2/1992           | Pittard et al.        | 5,707,214 A | 1/1998   | Schmidt                  |
| 5,095,988 A           | 3/1992           | Bode                  | 5,709,269 A | 1/1998   | Head                     |
|                       |                  |                       | 5,720,344 A | 2/1998   | Newman                   |
|                       |                  |                       | 5,722,033 A | 2/1998   | Carden                   |
|                       |                  |                       | 5,728,195 A | 3/1998   | Eastman et al.           |
|                       |                  |                       | 5,765,639 A | 6/1998   | Muth                     |

| (56)                  | References Cited |                    |              |         |                    |
|-----------------------|------------------|--------------------|--------------|---------|--------------------|
| U.S. PATENT DOCUMENTS |                  |                    |              |         |                    |
| 5,772,735 A           | 6/1998           | Sehgal et al.      | 6,397,950 B1 | 6/2002  | Streich et al.     |
| 5,782,305 A           | 7/1998           | Hicks              | 6,401,547 B1 | 6/2002  | Hatfield et al.    |
| 5,797,454 A           | 8/1998           | Hipp               | 6,403,210 B1 | 6/2002  | Stuivinga et al.   |
| 5,826,652 A           | 10/1998          | Tapp               | 6,408,946 B1 | 6/2002  | Marshall et al.    |
| 5,826,661 A           | 10/1998          | Parker et al.      | 6,419,023 B1 | 7/2002  | George et al.      |
| 5,829,520 A           | 11/1998          | Johnson            | 6,439,313 B1 | 8/2002  | Thomeer et al.     |
| 5,836,396 A           | 11/1998          | Norman             | 6,446,717 B1 | 9/2002  | White et al.       |
| 5,857,521 A           | 1/1999           | Ross et al.        | 6,457,525 B1 | 10/2002 | Scott              |
| 5,881,816 A           | 3/1999           | Wright             | 6,467,546 B2 | 10/2002 | Allamon et al.     |
| 5,896,819 A           | 4/1999           | Turila et al.      | 6,470,965 B1 | 10/2002 | Winzer             |
| 5,902,424 A           | 5/1999           | Fujita et al.      | 6,491,097 B1 | 12/2002 | Oneal et al.       |
| 5,934,372 A           | 8/1999           | Muth               | 6,491,116 B2 | 12/2002 | Berscheid et al.   |
| 5,941,309 A           | 8/1999           | Appleton           | 6,513,598 B2 | 2/2003  | Moore et al.       |
| 5,960,881 A           | 10/1999          | Allamon et al.     | 6,513,600 B2 | 2/2003  | Ross               |
| 5,964,965 A           | 10/1999          | Schulz et al.      | 6,540,033 B1 | 4/2003  | Sullivan et al.    |
| 5,985,466 A           | 11/1999          | Atarashi et al.    | 6,543,543 B2 | 4/2003  | Muth               |
| 5,988,287 A           | 11/1999          | Jordan, Jr. et al. | 6,561,275 B2 | 5/2003  | Glass et al.       |
| 5,990,051 A           | 11/1999          | Ischy et al.       | 6,588,507 B2 | 7/2003  | Dusterhoff et al.  |
| 5,992,452 A           | 11/1999          | Nelson, II         | 6,591,915 B2 | 7/2003  | Burris et al.      |
| 5,992,520 A           | 11/1999          | Schultz et al.     | 6,601,648 B2 | 8/2003  | Ebinger            |
| 6,007,314 A           | 12/1999          | Nelson, II         | 6,601,650 B2 | 8/2003  | Sundararajan       |
| 6,024,915 A           | 2/2000           | Kume et al.        | 6,609,569 B2 | 8/2003  | Howlett et al.     |
| 6,032,735 A           | 3/2000           | Echols             | 6,612,826 B1 | 9/2003  | Bauer et al.       |
| 6,036,777 A           | 3/2000           | Sachs              | 6,613,383 B1 | 9/2003  | George et al.      |
| 6,047,773 A           | 4/2000           | Zeltmann et al.    | 6,619,400 B2 | 9/2003  | Brunet             |
| 6,050,340 A           | 4/2000           | Scott              | 6,634,428 B2 | 10/2003 | Krauss et al.      |
| 6,069,313 A           | 5/2000           | Kay                | 6,662,886 B2 | 12/2003 | Russell            |
| 6,076,600 A           | 6/2000           | Vick, Jr. et al.   | 6,675,889 B1 | 1/2004  | Mullins et al.     |
| 6,079,496 A           | 6/2000           | Hirth              | 6,699,305 B2 | 3/2004  | Myrick             |
| 6,085,837 A           | 7/2000           | Massinon et al.    | 6,712,153 B2 | 3/2004  | Turley et al.      |
| 6,095,247 A           | 8/2000           | Streich et al.     | 6,712,797 B1 | 3/2004  | Southern, Jr.      |
| 6,119,783 A           | 9/2000           | Parker et al.      | 6,713,177 B2 | 3/2004  | George et al.      |
| 6,142,237 A           | 11/2000          | Christmas et al.   | 6,715,541 B2 | 4/2004  | Pedersen et al.    |
| 6,161,622 A           | 12/2000          | Robb               | 6,719,051 B2 | 4/2004  | Hailey, Jr. et al. |
| 6,167,970 B1          | 1/2001           | Stout et al.       | 6,755,249 B2 | 6/2004  | Robison et al.     |
| 6,170,583 B1          | 1/2001           | Boyce              | 6,769,491 B2 | 8/2004  | Zimmerman et al.   |
| 6,173,779 B1          | 1/2001           | Smith              | 6,776,228 B2 | 8/2004  | Pedersen et al.    |
| 6,176,323 B1          | 1/2001           | Weirich et al.     | 6,779,599 B2 | 8/2004  | Mullins et al.     |
| 6,189,616 B1          | 2/2001           | Gano et al.        | 6,799,638 B2 | 10/2004 | Butterfield, Jr.   |
| 6,189,618 B1          | 2/2001           | Beeman et al.      | 6,810,960 B2 | 11/2004 | Pia                |
| 6,213,202 B1          | 4/2001           | Read, Jr.          | 6,817,414 B2 | 11/2004 | Lee                |
| 6,220,350 B1          | 4/2001           | Brothers et al.    | 6,831,044 B2 | 12/2004 | Constien           |
| 6,220,357 B1          | 4/2001           | Carmichael et al.  | 6,883,611 B2 | 4/2005  | Smith et al.       |
| 6,228,904 B1          | 5/2001           | Yadav et al.       | 6,887,297 B2 | 5/2005  | Winter et al.      |
| 6,237,688 B1          | 5/2001           | Burleson et al.    | 6,908,516 B2 | 6/2005  | Hehmann et al.     |
| 6,238,280 B1          | 5/2001           | Ritt et al.        | 6,913,827 B2 | 7/2005  | George et al.      |
| 6,241,021 B1          | 6/2001           | Bowling            | 6,926,086 B2 | 8/2005  | Patterson et al.   |
| 6,248,399 B1          | 6/2001           | Hehmann            | 6,932,159 B2 | 8/2005  | Hovem              |
| 6,250,392 B1          | 6/2001           | Muth               | 6,939,388 B2 | 9/2005  | Angeliu            |
| 6,261,432 B1          | 7/2001           | Huber et al.       | 6,945,331 B2 | 9/2005  | Patel              |
| 6,265,205 B1          | 7/2001           | Hitchens et al.    | 6,951,331 B2 | 10/2005 | Haughom et al.     |
| 6,273,187 B1          | 8/2001           | Voisin, Jr. et al. | 6,959,759 B2 | 11/2005 | Doane et al.       |
| 6,276,452 B1          | 8/2001           | Davis et al.       | 6,973,970 B2 | 12/2005 | Johnston et al.    |
| 6,276,457 B1          | 8/2001           | Moffatt et al.     | 6,973,973 B2 | 12/2005 | Howard et al.      |
| 6,279,656 B1          | 8/2001           | Sinclair et al.    | 6,983,796 B2 | 1/2006  | Bayne et al.       |
| 6,287,445 B1          | 9/2001           | Lashmore et al.    | 6,986,390 B2 | 1/2006  | Doane et al.       |
| 6,302,205 B1          | 10/2001          | Ryll               | 7,013,989 B2 | 3/2006  | Hammond et al.     |
| 6,315,041 B1          | 11/2001          | Carlisle et al.    | 7,013,998 B2 | 3/2006  | Ray et al.         |
| 6,315,050 B2          | 11/2001          | Vaynshteyn et al.  | 7,017,664 B2 | 3/2006  | Walker et al.      |
| 6,325,148 B1          | 12/2001          | Trahan et al.      | 7,017,677 B2 | 3/2006  | Keshavan et al.    |
| 6,328,110 B1          | 12/2001          | Joubert            | 7,021,389 B2 | 4/2006  | Bishop et al.      |
| 6,341,653 B1          | 1/2002           | Firmaniuk et al.   | 7,025,146 B2 | 4/2006  | King et al.        |
| 6,341,747 B1          | 1/2002           | Schmidt et al.     | 7,028,778 B2 | 4/2006  | Krywitsky          |
| 6,349,766 B1          | 2/2002           | Bussear et al.     | 7,044,230 B2 | 5/2006  | Starr et al.       |
| 6,354,372 B1          | 3/2002           | Carisella et al.   | 7,049,272 B2 | 5/2006  | Sinclair et al.    |
| 6,354,379 B2          | 3/2002           | Miszewski et al.   | 7,051,805 B2 | 5/2006  | Doane et al.       |
| 6,357,322 B1          | 3/2002           | Dolan et al.       | 7,059,410 B2 | 6/2006  | Bousche et al.     |
| 6,357,332 B1          | 3/2002           | Vecchio            | 7,090,027 B1 | 8/2006  | Williams           |
| 6,371,206 B1          | 4/2002           | Mills              | 7,093,664 B2 | 8/2006  | Todd et al.        |
| 6,372,346 B1          | 4/2002           | Toth               | 7,096,945 B2 | 8/2006  | Richards et al.    |
| 6,382,244 B2          | 5/2002           | Vann               | 7,096,946 B2 | 8/2006  | Jasser et al.      |
| 6,390,195 B1          | 5/2002           | Nguyen et al.      | 7,097,807 B1 | 8/2006  | Meeks, III et al.  |
| 6,390,200 B1          | 5/2002           | Allamon et al.     | 7,097,906 B2 | 8/2006  | Gardner            |
| 6,394,180 B1          | 5/2002           | Berscheid et al.   | 7,108,080 B2 | 9/2006  | Tessari et al.     |
| 6,394,185 B1          | 5/2002           | Constien           | 7,111,682 B2 | 9/2006  | Blaisdell          |

# US 10,016,810 B2

Page 4

---

(56)

## References Cited

### U.S. PATENT DOCUMENTS

|              |         |                          |              |         |                     |
|--------------|---------|--------------------------|--------------|---------|---------------------|
| 7,128,145 B2 | 10/2006 | Mickey                   | 7,661,481 B2 | 2/2010  | Todd et al.         |
| 7,141,207 B2 | 11/2006 | Jandeska, Jr. et al.     | 7,665,537 B2 | 2/2010  | Patel et al.        |
| 7,150,326 B2 | 12/2006 | Bishop et al.            | 7,686,082 B2 | 3/2010  | Marsh               |
| 7,163,066 B2 | 1/2007  | Lehr                     | 7,690,436 B2 | 4/2010  | Turley et al.       |
| 7,165,622 B2 | 1/2007  | Hirth et al.             | 7,699,101 B2 | 4/2010  | Fripp et al.        |
| 7,168,494 B2 | 1/2007  | Starr et al.             | 7,703,510 B2 | 4/2010  | Xu                  |
| 7,174,963 B2 | 2/2007  | Bertelsen                | 7,703,511 B2 | 4/2010  | Buyers et al.       |
| 7,182,135 B2 | 2/2007  | Szarka                   | 7,712,541 B2 | 5/2010  | Loretz et al.       |
| 7,188,559 B1 | 3/2007  | Vecchio                  | 7,723,272 B2 | 5/2010  | Crews et al.        |
| 7,210,527 B2 | 5/2007  | Walker et al.            | 7,726,406 B2 | 6/2010  | Xu                  |
| 7,210,533 B2 | 5/2007  | Starr et al.             | 7,735,578 B2 | 6/2010  | Loehr et al.        |
| 7,217,311 B2 | 5/2007  | Hong et al.              | 7,743,836 B2 | 6/2010  | Cook et al.         |
| 7,234,530 B2 | 6/2007  | Gass                     | 7,752,971 B2 | 7/2010  | Loehr               |
| 7,250,188 B2 | 7/2007  | Dodelet et al.           | 7,757,773 B2 | 7/2010  | Rytlewski           |
| 7,252,162 B2 | 8/2007  | Akinlade et al.          | 7,762,342 B2 | 7/2010  | Richard et al.      |
| 7,255,172 B2 | 8/2007  | Johnson                  | 7,770,652 B2 | 8/2010  | Barnett             |
| 7,255,178 B2 | 8/2007  | Slup et al.              | 7,771,289 B2 | 8/2010  | Palumbo et al.      |
| 7,264,060 B2 | 9/2007  | Wills                    | 7,775,284 B2 | 8/2010  | Richards et al.     |
| 7,267,172 B2 | 9/2007  | Hofman                   | 7,775,285 B2 | 8/2010  | Surjaatmadja et al. |
| 7,267,178 B2 | 9/2007  | Krywitsky                | 7,775,286 B2 | 8/2010  | Duphorne            |
| 7,270,186 B2 | 9/2007  | Johnson                  | 7,784,543 B2 | 8/2010  | Johnson             |
| 7,287,592 B2 | 10/2007 | Surjaatmadja et al.      | 7,806,189 B2 | 10/2010 | Frazier             |
| 7,311,152 B2 | 12/2007 | Howard et al.            | 7,806,192 B2 | 10/2010 | Foster et al.       |
| 7,316,274 B2 | 1/2008  | Xu et al.                | 7,810,553 B2 | 10/2010 | Cruickshank et al.  |
| 7,320,365 B2 | 1/2008  | Pia                      | 7,810,567 B2 | 10/2010 | Daniels et al.      |
| 7,322,412 B2 | 1/2008  | Badalamenti et al.       | 7,819,198 B2 | 10/2010 | Birckhead et al.    |
| 7,322,417 B2 | 1/2008  | Rytlewski et al.         | 7,828,055 B2 | 11/2010 | Willauer et al.     |
| 7,325,617 B2 | 2/2008  | Murray                   | 7,833,944 B2 | 11/2010 | Munoz et al.        |
| 7,328,750 B2 | 2/2008  | Swor et al.              | 7,849,927 B2 | 12/2010 | Herrera             |
| 7,331,388 B2 | 2/2008  | Vilela et al.            | 7,851,016 B2 | 12/2010 | Arbab et al.        |
| 7,337,854 B2 | 3/2008  | Horn et al.              | 7,855,168 B2 | 12/2010 | Fuller et al.       |
| 7,346,456 B2 | 3/2008  | Le Bemadjel              | 7,861,779 B2 | 1/2011  | Vestavik            |
| 7,350,582 B2 | 4/2008  | McKeachnie et al.        | 7,861,781 B2 | 1/2011  | D'Arcy              |
| 7,353,879 B2 | 4/2008  | Todd et al.              | 7,874,365 B2 | 1/2011  | East, Jr. et al.    |
| 7,360,593 B2 | 4/2008  | Constien                 | 7,878,253 B2 | 2/2011  | Stowe et al.        |
| 7,360,597 B2 | 4/2008  | Blaisdell                | 7,879,367 B2 | 2/2011  | Heublein et al.     |
| 7,363,970 B2 | 4/2008  | Corre et al.             | 7,896,091 B2 | 3/2011  | Williamson et al.   |
| 7,373,978 B2 | 5/2008  | Barry et al.             | 7,897,063 B1 | 3/2011  | Perry et al.        |
| 7,384,443 B2 | 6/2008  | Mirchandani              | 7,900,696 B1 | 3/2011  | Nish et al.         |
| 7,387,158 B2 | 6/2008  | Murray et al.            | 7,900,703 B2 | 3/2011  | Clark et al.        |
| 7,387,165 B2 | 6/2008  | Lopez De Cardenas et al. | 7,909,096 B2 | 3/2011  | Clark et al.        |
| 7,392,841 B2 | 7/2008  | Murray et al.            | 7,909,104 B2 | 3/2011  | Bjorgum             |
| 7,401,648 B2 | 7/2008  | Bennett                  | 7,909,110 B2 | 3/2011  | Sharma et al.       |
| 7,416,029 B2 | 8/2008  | Telfer et al.            | 7,909,115 B2 | 3/2011  | Grove et al.        |
| 7,422,058 B2 | 9/2008  | O'Malley                 | 7,913,765 B2 | 3/2011  | Crow et al.         |
| 7,426,964 B2 | 9/2008  | Lynde et al.             | 7,918,275 B2 | 4/2011  | Clem                |
| 7,441,596 B2 | 10/2008 | Wood et al.              | 7,931,093 B2 | 4/2011  | Foster et al.       |
| 7,445,049 B2 | 11/2008 | Howard et al.            | 7,938,191 B2 | 5/2011  | Vaidya              |
| 7,451,815 B2 | 11/2008 | Hailey, Jr.              | 7,946,335 B2 | 5/2011  | Bewlay et al.       |
| 7,451,817 B2 | 11/2008 | Reddy et al.             | 7,946,340 B2 | 5/2011  | Surjaatmadja et al. |
| 7,461,699 B2 | 12/2008 | Richard et al.           | 7,958,940 B2 | 6/2011  | Jameson             |
| 7,464,764 B2 | 12/2008 | Xu                       | 7,963,331 B2 | 6/2011  | Surjaatmadja et al. |
| 7,472,750 B2 | 1/2009  | Walker et al.            | 7,963,340 B2 | 6/2011  | Gramstad et al.     |
| 7,478,676 B2 | 1/2009  | East, Jr. et al.         | 7,963,342 B2 | 6/2011  | George              |
| 7,503,390 B2 | 3/2009  | Gomez                    | 7,980,300 B2 | 7/2011  | Roberts et al.      |
| 7,503,399 B2 | 3/2009  | Badalamenti et al.       | 7,987,906 B1 | 8/2011  | Troy                |
| 7,509,993 B1 | 3/2009  | Turng et al.             | 7,992,763 B2 | 8/2011  | Vecchio et al.      |
| 7,510,018 B2 | 3/2009  | Williamson et al.        | 8,020,619 B1 | 9/2011  | Robertson et al.    |
| 7,513,311 B2 | 4/2009  | Gramstad et al.          | 8,020,620 B2 | 9/2011  | Daniels et al.      |
| 7,527,103 B2 | 5/2009  | Huang et al.             | 8,025,104 B2 | 9/2011  | Cooke, Jr.          |
| 7,537,825 B1 | 5/2009  | Wardle et al.            | 8,028,767 B2 | 10/2011 | Radford et al.      |
| 7,552,777 B2 | 6/2009  | Murray et al.            | 8,033,331 B2 | 10/2011 | Themig              |
| 7,552,779 B2 | 6/2009  | Murray                   | 8,039,422 B1 | 10/2011 | Al-Zahrani          |
| 7,559,357 B2 | 7/2009  | Clem                     | 8,056,628 B2 | 11/2011 | Whitsitt et al.     |
| 7,575,062 B2 | 8/2009  | East, Jr.                | 8,056,638 B2 | 11/2011 | Clayton et al.      |
| 7,579,087 B2 | 8/2009  | Maloney et al.           | 8,109,340 B2 | 2/2012  | Doane et al.        |
| 7,591,318 B2 | 9/2009  | Tilghman                 | 8,127,856 B1 | 3/2012  | Nish et al.         |
| 7,600,572 B2 | 10/2009 | Slup et al.              | 8,163,060 B2 | 4/2012  | Imanishi et al.     |
| 7,604,049 B2 | 10/2009 | Vaidya et al.            | 8,211,247 B2 | 7/2012  | Marya et al.        |
| 7,604,055 B2 | 10/2009 | Richard et al.           | 8,211,248 B2 | 7/2012  | Marya               |
| 7,607,476 B2 | 10/2009 | Tom et al.               | 8,220,554 B2 | 7/2012  | Jordan et al.       |
| 7,617,871 B2 | 11/2009 | Surjaatmadja et al.      | 8,226,740 B2 | 7/2012  | Chaumonnot et al.   |
| 7,635,023 B2 | 12/2009 | Goldberg et al.          | 8,230,731 B2 | 7/2012  | Dyer et al.         |
| 7,640,988 B2 | 1/2010  | Phi et al.               | 8,231,947 B2 | 7/2012  | Vaidya et al.       |
| 7,661,480 B2 | 2/2010  | Al-Anazi                 |              |         |                     |

| (56)                  | References Cited |         |                      |              |    |              |                          |
|-----------------------|------------------|---------|----------------------|--------------|----|--------------|--------------------------|
| U.S. PATENT DOCUMENTS |                  |         |                      |              |    |              |                          |
| 8,263,178             | B2               | 9/2012  | Boulos et al.        | 2004/0231845 | A1 | 11/2004      | Cooke, Jr.               |
| 8,276,670             | B2               | 10/2012 | Patel                | 2004/0251025 | A1 | 12/2004      | Giroux et al.            |
| 8,277,974             | B2               | 10/2012 | Kumar et al.         | 2005/0034876 | A1 | 2/2005       | Doane et al.             |
| 8,297,364             | B2               | 10/2012 | Agrawal et al.       | 2005/0051329 | A1 | 3/2005       | Blaisdell                |
| 8,327,931             | B2               | 12/2012 | Agrawal et al.       | 2005/0064247 | A1 | 3/2005       | Sane                     |
| 8,403,037             | B2               | 3/2013  | Agrawal et al.       | 2005/0069449 | A1 | 3/2005       | Jackson et al.           |
| 8,413,727             | B2               | 4/2013  | Holmes               | 2005/0074612 | A1 | 4/2005       | Eklund et al.            |
| 8,425,651             | B2 *             | 4/2013  | Xu .....             | B22F 1/025   |    | 2005/0098313 | A1                       |
|                       |                  |         |                      | 75/245       |    | 2005/0102255 | A1                       |
|                       |                  |         |                      |              |    | 5/2005       | Bultman                  |
| 8,459,347             | B2               | 6/2013  | Stout                | 2005/0106316 | A1 | 5/2005       | Rigney et al.            |
| 8,486,329             | B2               | 7/2013  | Shikai et al.        | 2005/0126334 | A1 | 6/2005       | Mirchandani              |
| 8,490,674             | B2               | 7/2013  | Stevens et al.       | 2005/0161212 | A1 | 7/2005       | Leismer et al.           |
| 8,490,689             | B1               | 7/2013  | McClinton et al.     | 2005/0161224 | A1 | 7/2005       | Starr et al.             |
| 8,535,604             | B1               | 9/2013  | Baker et al.         | 2005/0165149 | A1 | 7/2005       | Chanak et al.            |
| 8,573,295             | B2               | 11/2013 | Johnson et al.       | 2005/0194143 | A1 | 9/2005       | Xu et al.                |
| 8,631,876             | B2               | 1/2014  | Xu et al.            | 2005/0199401 | A1 | 9/2005       | Patel et al.             |
| 8,663,401             | B2               | 3/2014  | Marya et al.         | 2005/0205264 | A1 | 9/2005       | Starr et al.             |
| 8,734,602             | B2               | 5/2014  | Li et al.            | 2005/0205265 | A1 | 9/2005       | Todd et al.              |
| 8,770,261             | B2               | 7/2014  | Marya                | 2005/0205266 | A1 | 9/2005       | Todd et al.              |
| 8,956,660             | B2               | 2/2015  | Launag et al.        | 2005/0235757 | A1 | 10/2005      | De Jonge et al.          |
| 8,978,734             | B2               | 3/2015  | Stevens              | 2005/0241824 | A1 | 11/2005      | Burris, II et al.        |
| 8,998,978             | B2               | 4/2015  | Wang                 | 2005/0241825 | A1 | 11/2005      | Burris, II et al.        |
| 9,057,242             | B2               | 6/2015  | Mazyar et al.        | 2005/0257936 | A1 | 11/2005      | Lehr                     |
| 9,079,246             | B2               | 7/2015  | Xu et al.            | 2005/0268746 | A1 | 12/2005      | Abkowitz et al.          |
| 9,080,098             | B2               | 7/2015  | Xu et al.            | 2005/0269097 | A1 | 12/2005      | Towler                   |
| 9,089,408             | B2               | 7/2015  | Xu                   | 2005/0275143 | A1 | 12/2005      | Toth                     |
| 9,090,955             | B2               | 7/2015  | Xu et al.            | 2005/0279501 | A1 | 12/2005      | Surjaatmadja et al.      |
| 9,243,475             | B2               | 1/2016  | Xu                   | 2006/0012087 | A1 | 1/2006       | Matsuda et al.           |
| 9,260,935             | B2               | 2/2016  | Murphree et al.      | 2006/0013350 | A1 | 1/2006       | Akers                    |
| 2001/0040180          | A1               | 11/2001 | Wittebrood et al.    | 2006/0045787 | A1 | 3/2006       | Jandeska et al.          |
| 2001/0045285          | A1               | 11/2001 | Russell              | 2006/0057479 | A1 | 3/2006       | Niimi et al.             |
| 2001/0045288          | A1               | 11/2001 | Allamon et al.       | 2006/0081378 | A1 | 4/2006       | Howard et al.            |
| 2002/0000319          | A1               | 1/2002  | Brunet               | 2006/0102871 | A1 | 5/2006       | Wang                     |
| 2002/0007948          | A1               | 1/2002  | Bayne et al.         | 2006/0108114 | A1 | 5/2006       | Johnson et al.           |
| 2002/0014268          | A1               | 2/2002  | Vann                 | 2006/0108126 | A1 | 5/2006       | Horn et al.              |
| 2002/0020527          | A1               | 2/2002  | Kilaas et al.        | 2006/0110615 | A1 | 5/2006       | Karim et al.             |
| 2002/0066572          | A1               | 6/2002  | Muth                 | 2006/0116696 | A1 | 6/2006       | Odermatt et al.          |
| 2002/0092654          | A1               | 7/2002  | Coronado et al.      | 2006/0124310 | A1 | 6/2006       | Lopez De Cardenas et al. |
| 2002/0096365          | A1               | 7/2002  | Berscheidt et al.    | 2006/0131011 | A1 | 6/2006       | Lynde et al.             |
| 2002/0104616          | A1               | 8/2002  | De et al.            | 2006/0131031 | A1 | 6/2006       | McKeachnie et al.        |
| 2002/0108756          | A1               | 8/2002  | Harrall et al.       | 2006/0131081 | A1 | 6/2006       | Mirchandani et al.       |
| 2002/0136904          | A1               | 9/2002  | Glass et al.         | 2006/0134312 | A1 | 6/2006       | Rytlewski et al.         |
| 2002/0139541          | A1               | 10/2002 | Sheffield et al.     | 2006/0144515 | A1 | 7/2006       | Tada et al.              |
| 2002/0162661          | A1               | 11/2002 | Krauss et al.        | 2006/0150770 | A1 | 7/2006       | Freim                    |
| 2003/0019639          | A1               | 1/2003  | MacKay               | 2006/0151178 | A1 | 7/2006       | Howard et al.            |
| 2003/0037925          | A1               | 2/2003  | Walker et al.        | 2006/0153728 | A1 | 7/2006       | Schoenung et al.         |
| 2003/0060374          | A1               | 3/2003  | Cooke, Jr.           | 2006/0162927 | A1 | 7/2006       | Walker et al.            |
| 2003/0075326          | A1               | 4/2003  | Ebinger              | 2006/0169453 | A1 | 8/2006       | Savery et al.            |
| 2003/0104147          | A1               | 6/2003  | Bretschneider et al. | 2006/0186602 | A1 | 8/2006       | Martin et al.            |
| 2003/0111728          | A1               | 6/2003  | Thai et al.          | 2006/0207763 | A1 | 9/2006       | Hofman et al.            |
| 2003/0127013          | A1               | 7/2003  | Zavitsanos et al.    | 2006/0213670 | A1 | 9/2006       | Bishop et al.            |
| 2003/0141060          | A1               | 7/2003  | Hailey et al.        | 2006/0231253 | A1 | 10/2006      | Vilela et al.            |
| 2003/0141061          | A1               | 7/2003  | Hailey et al.        | 2006/0269437 | A1 | 11/2006      | Pandey                   |
| 2003/0141079          | A1               | 7/2003  | Doane et al.         | 2006/0283592 | A1 | 12/2006      | Sierra et al.            |
| 2003/0150614          | A1               | 8/2003  | Brown et al.         | 2007/0017674 | A1 | 1/2007       | Blaisdell                |
| 2003/0155114          | A1               | 8/2003  | Pedersen et al.      | 2007/0017675 | A1 | 1/2007       | Hammami                  |
| 2003/0155115          | A1               | 8/2003  | Pedersen et al.      | 2007/0029082 | A1 | 2/2007       | Giroux et al.            |
| 2003/0159828          | A1               | 8/2003  | Howard et al.        | 2007/0039161 | A1 | 2/2007       | Garcia                   |
| 2003/0164237          | A1               | 9/2003  | Butterfield          | 2007/0039741 | A1 | 2/2007       | Hailey                   |
| 2003/0183391          | A1               | 10/2003 | Hriscu et al.        | 2007/0044958 | A1 | 3/2007       | Rytlewski et al.         |
| 2003/0226668          | A1               | 12/2003 | Zimmerman et al.     | 2007/0044966 | A1 | 3/2007       | Davies et al.            |
| 2004/0005483          | A1               | 1/2004  | Lin                  | 2007/0051521 | A1 | 3/2007       | Fike et al.              |
| 2004/0020832          | A1               | 2/2004  | Richards et al.      | 2007/0053785 | A1 | 3/2007       | Hetz et al.              |
| 2004/0031605          | A1               | 2/2004  | Mickey               | 2007/0054101 | A1 | 3/2007       | McKeachnie et al.        |
| 2004/0045723          | A1               | 3/2004  | Slup et al.          | 2007/0057415 | A1 | 3/2007       | Katagiri et al.          |
| 2004/0055758          | A1               | 3/2004  | Brezinski et al.     | 2007/0062644 | A1 | 3/2007       | Nakamura et al.          |
| 2004/0058167          | A1               | 3/2004  | Arbab et al.         | 2007/0074601 | A1 | 4/2007       | Hong et al.              |
| 2004/0069502          | A1               | 4/2004  | Luke                 | 2007/0074873 | A1 | 4/2007       | McKeachnie et al.        |
| 2004/0089449          | A1               | 5/2004  | Walton et al.        | 2007/0102199 | A1 | 5/2007       | Smith et al.             |
| 2004/0094297          | A1               | 5/2004  | Malone et al.        | 2007/0107899 | A1 | 5/2007       | Werner et al.            |
| 2004/0154806          | A1               | 8/2004  | Bode et al.          | 2007/0107908 | A1 | 5/2007       | Vaidya et al.            |
| 2004/0159428          | A1               | 8/2004  | Hammond et al.       | 2007/0108060 | A1 | 5/2007       | Park                     |
| 2004/0159446          | A1               | 8/2004  | Haugen et al.        | 2007/0119600 | A1 | 5/2007       | Slup et al.              |
| 2004/0182583          | A1               | 9/2004  | Doane et al.         | 2007/0131912 | A1 | 6/2007       | Simone et al.            |
| 2004/0216868          | A1               | 11/2004 | Owen, Sr.            | 2007/0151009 | A1 | 7/2007       | Conrad, III et al.       |

| (56)                  | References Cited |                          |                  |         |                          |             |
|-----------------------|------------------|--------------------------|------------------|---------|--------------------------|-------------|
| U.S. PATENT DOCUMENTS |                  |                          |                  |         |                          |             |
| 2007/0151769 A1       | 7/2007           | Slutz et al.             | 2009/0139720 A1  | 6/2009  | Frazier                  |             |
| 2007/0169935 A1       | 7/2007           | Akbar et al.             | 2009/0145666 A1  | 6/2009  | Radford et al.           |             |
| 2007/0181224 A1       | 8/2007           | Marya et al.             | 2009/0151949 A1  | 6/2009  | Marya et al.             |             |
| 2007/0185655 A1       | 8/2007           | Le Bemadjiel             | 2009/0152009 A1  | 6/2009  | Slay et al.              |             |
| 2007/0187095 A1       | 8/2007           | Walker et al.            | 2009/0155616 A1  | 6/2009  | Thamida et al.           |             |
| 2007/0207182 A1       | 9/2007           | Weber et al.             | 2009/0159289 A1  | 6/2009  | Avant et al.             |             |
| 2007/0221373 A1       | 9/2007           | Murray                   | 2009/0178808 A1  | 7/2009  | Williamson et al.        |             |
| 2007/0221384 A1       | 9/2007           | Murray                   | 2009/0194273 A1  | 8/2009  | Surjaatmadja et al.      |             |
| 2007/0227745 A1       | 10/2007          | Roberts et al.           | 2009/0194745 A1* | 8/2009  | Tanaka .....             | B23K 35/262 |
| 2007/0259994 A1       | 11/2007          | Tour et al.              |                  |         |                          | 252/514     |
| 2007/0261862 A1       | 11/2007          | Murray                   | 2009/0205841 A1  | 8/2009  | Kluge et al.             |             |
| 2007/0272411 A1       | 11/2007          | Lopez De Cardenas et al. | 2009/0211770 A1  | 8/2009  | Nutley et al.            |             |
| 2007/0272413 A1       | 11/2007          | Rytlewski et al.         | 2009/0226340 A1  | 9/2009  | Marya                    |             |
| 2007/0277979 A1       | 12/2007          | Todd et al.              | 2009/0226704 A1  | 9/2009  | Kauppinen et al.         |             |
| 2007/0284109 A1       | 12/2007          | East et al.              | 2009/0242202 A1  | 10/2009 | Rispler et al.           |             |
| 2007/0284112 A1       | 12/2007          | Magne et al.             | 2009/0242208 A1  | 10/2009 | Bolding                  |             |
| 2007/0299510 A1       | 12/2007          | Venkatraman et al.       | 2009/0242214 A1  | 10/2009 | Foster et al.            |             |
| 2008/0011473 A1       | 1/2008           | Wood et al.              | 2009/0255667 A1  | 10/2009 | Clem et al.              |             |
| 2008/0020923 A1       | 1/2008           | Debe et al.              | 2009/0255684 A1  | 10/2009 | Bolding                  |             |
| 2008/0047707 A1       | 2/2008           | Boney et al.             | 2009/0255686 A1  | 10/2009 | Richard                  |             |
| 2008/0060810 A9       | 3/2008           | Nguyen et al.            | 2009/0266548 A1  | 10/2009 | Olsen et al.             |             |
| 2008/0066923 A1       | 3/2008           | Xu                       | 2009/0260817 A1  | 11/2009 | Gambier et al.           |             |
| 2008/0066924 A1       | 3/2008           | Xu                       | 2009/0272544 A1  | 11/2009 | Giroux et al.            |             |
| 2008/0072705 A1       | 3/2008           | Chaumonnot et al.        | 2009/0283270 A1  | 11/2009 | Langeslag                |             |
| 2008/0078553 A1       | 4/2008           | George                   | 2009/0293672 A1  | 12/2009 | Mirchandani et al.       |             |
| 2008/0081866 A1       | 4/2008           | Gong et al.              | 2009/0301730 A1  | 12/2009 | Gweily                   |             |
| 2008/0093073 A1       | 4/2008           | Bustos et al.            | 2009/0305131 A1  | 12/2009 | Kumar et al.             |             |
| 2008/0099209 A1       | 5/2008           | Loretz et al.            | 2009/0308588 A1  | 12/2009 | Howell et al.            |             |
| 2008/0105438 A1       | 5/2008           | Jordan et al.            | 2009/0317556 A1  | 12/2009 | Macary                   |             |
| 2008/0115932 A1       | 5/2008           | Cooke                    | 2009/0317622 A1  | 12/2009 | Huang et al.             |             |
| 2008/0121390 A1       | 5/2008           | O'Malley et al.          | 2010/0003536 A1  | 1/2010  | Smith et al.             |             |
| 2008/0121436 A1       | 5/2008           | Slay et al.              | 2010/0012385 A1  | 1/2010  | Drivdahl et al.          |             |
| 2008/0127475 A1       | 6/2008           | Griffo                   | 2010/0015002 A1  | 1/2010  | Barrera et al.           |             |
| 2008/0135249 A1       | 6/2008           | Fripp et al.             | 2010/0015469 A1  | 1/2010  | Romanowski et al.        |             |
| 2008/0149325 A1       | 6/2008           | Crawford                 | 2010/0025255 A1  | 2/2010  | Su et al.                |             |
| 2008/0149345 A1       | 6/2008           | Bicerano                 | 2010/0032151 A1  | 2/2010  | Duphorne et al.          |             |
| 2008/0149351 A1       | 6/2008           | Marya et al.             | 2010/0034857 A1  | 2/2010  | Launag et al.            |             |
| 2008/0169105 A1       | 7/2008           | Williamson et al.        | 2010/0038076 A1  | 2/2010  | Spray et al.             |             |
| 2008/0169130 A1       | 7/2008           | Norman et al.            | 2010/0038595 A1  | 2/2010  | Imholt et al.            |             |
| 2008/0179060 A1       | 7/2008           | Surjaatmadja et al.      | 2010/0040180 A1  | 2/2010  | Kim et al.               |             |
| 2008/0179104 A1       | 7/2008           | Zhang et al.             | 2010/0044041 A1  | 2/2010  | Smith et al.             |             |
| 2008/0196801 A1       | 8/2008           | Zhao et al.              | 2010/0051278 A1  | 3/2010  | Mytopher et al.          |             |
| 2008/0202764 A1       | 8/2008           | Clayton et al.           | 2010/0055491 A1  | 3/2010  | Vecchio et al.           |             |
| 2008/0202814 A1       | 8/2008           | Lyons et al.             | 2010/0055492 A1  | 3/2010  | Barsoum et al.           |             |
| 2008/0210473 A1       | 9/2008           | Zhang et al.             | 2010/0089583 A1  | 4/2010  | Xu et al.                |             |
| 2008/0216383 A1       | 9/2008           | Pierick et al.           | 2010/0089587 A1  | 4/2010  | Stout                    |             |
| 2008/0223586 A1       | 9/2008           | Barnett                  | 2010/0101803 A1  | 4/2010  | Clayton et al.           |             |
| 2008/0223587 A1       | 9/2008           | Cherewyk                 | 2010/0116495 A1  | 5/2010  | Spray                    |             |
| 2008/0236829 A1       | 10/2008          | Lynde                    | 2010/0122817 A1  | 5/2010  | Surjaatmadja et al.      |             |
| 2008/0236842 A1       | 10/2008          | Bhavsar et al.           | 2010/0139930 A1  | 6/2010  | Patel et al.             |             |
| 2008/0248205 A1       | 10/2008          | Blanchet et al.          | 2010/0200230 A1  | 8/2010  | East, Jr. et al.         |             |
| 2008/0248413 A1       | 10/2008          | Ishii et al.             | 2010/0209288 A1  | 8/2010  | Marya                    |             |
| 2008/0264594 A1       | 10/2008          | Lohmueller et al.        | 2010/0236793 A1  | 9/2010  | Bjorgum                  |             |
| 2008/0277109 A1       | 11/2008          | Vaidya                   | 2010/0236794 A1  | 9/2010  | Duan et al.              |             |
| 2008/0277980 A1       | 11/2008          | Koda et al.              | 2010/0243254 A1  | 9/2010  | Murphy et al.            |             |
| 2008/0282924 A1       | 11/2008          | Saenger et al.           | 2010/0252273 A1  | 10/2010 | Duphorne                 |             |
| 2008/0296024 A1       | 12/2008          | Tianping et al.          | 2010/0252280 A1  | 10/2010 | Swor et al.              |             |
| 2008/0302538 A1       | 12/2008          | Hofman                   | 2010/0270031 A1  | 10/2010 | Patel                    |             |
| 2008/0314581 A1       | 12/2008          | Brown                    | 2010/0276136 A1  | 11/2010 | Evans et al.             |             |
| 2008/0314588 A1       | 12/2008          | Langlais et al.          | 2010/0276159 A1  | 11/2010 | Mailand et al.           |             |
| 2009/0038858 A1       | 2/2009           | Griffo et al.            | 2010/0282338 A1  | 11/2010 | Gerrard et al.           |             |
| 2009/0044946 A1       | 2/2009           | Schasteen et al.         | 2010/0284269 A1  | 11/2010 | Richard et al.           |             |
| 2009/0044949 A1       | 2/2009           | King et al.              | 2010/0294510 A1  | 11/2010 | Holmes                   |             |
| 2009/0050334 A1       | 2/2009           | Marya et al.             | 2010/0297432 A1  | 11/2010 | Sherman et al.           |             |
| 2009/0056934 A1       | 3/2009           | Xu                       | 2010/0304182 A1  | 12/2010 | Facchini et al.          |             |
| 2009/0065216 A1       | 3/2009           | Frazier                  | 2010/0314105 A1  | 12/2010 | Rose                     |             |
| 2009/0074603 A1       | 3/2009           | Chan et al.              | 2010/0314126 A1  | 12/2010 | Kellner                  |             |
| 2009/0084553 A1       | 4/2009           | Rytlewski et al.         | 2010/0319870 A1  | 12/2010 | Bewlay et al.            |             |
| 2009/0084556 A1       | 4/2009           | Richards et al.          | 2010/0326650 A1  | 12/2010 | Tran et al.              |             |
| 2009/0084600 A1       | 4/2009           | Severance                | 2011/0005573 A1  | 1/2011  | Dusterhoff et al.        |             |
| 2009/0090440 A1       | 4/2009           | Kellett et al.           | 2011/0036592 A1  | 2/2011  | Fay                      |             |
| 2009/0107684 A1       | 4/2009           | Cooke, Jr.               | 2011/0048743 A1  | 3/2011  | Stafford et al.          |             |
| 2009/0114381 A1       | 5/2009           | Stroobants               | 2011/0052805 A1  | 3/2011  | Bordere et al.           |             |
| 2009/0114382 A1       | 5/2009           | Grove et al.             | 2011/0056692 A1  | 3/2011  | Lopez De Cardenas et al. |             |
| 2009/0126436 A1       | 5/2009           | Fly et al.               | 2011/0056702 A1  | 3/2011  | Sharma et al.            |             |
|                       |                  |                          | 2011/0067872 A1  | 3/2011  | Agrawal                  |             |
|                       |                  |                          | 2011/0067889 A1  | 3/2011  | Marya et al.             |             |
|                       |                  |                          | 2011/0067890 A1  | 3/2011  | Themig                   |             |
|                       |                  |                          | 2011/0094406 A1  | 4/2011  | Marya et al.             |             |

# US 10,016,810 B2

Page 7

(56)

## References Cited

### U.S. PATENT DOCUMENTS

|                  |         |                     |                 |         |                |
|------------------|---------|---------------------|-----------------|---------|----------------|
| 2011/0100643 A1  | 5/2011  | Themig et al.       | 2014/0116711 A1 | 5/2014  | Tang et al.    |
| 2011/0127044 A1  | 6/2011  | Radford et al.      | 2014/0186207 A1 | 7/2014  | Bae et al.     |
| 2011/0132143 A1  | 6/2011  | Xu et al.           | 2014/0190705 A1 | 7/2014  | Fripp et al.   |
| 2011/0132612 A1  | 6/2011  | Agrawal et al.      | 2014/0196899 A1 | 7/2014  | Jordan et al.  |
| 2011/0132619 A1  | 6/2011  | Agrawal et al.      | 2014/0262327 A1 | 9/2014  | Xu et al.      |
| 2011/0132620 A1  | 6/2011  | Agrawal et al.      | 2014/0360728 A1 | 12/2014 | Tashiro et al. |
| 2011/0132621 A1  | 6/2011  | Agrawal et al.      | 2015/0060085 A1 | 3/2015  | Xu             |
| 2011/0135530 A1  | 6/2011  | Xu et al.           | 2015/0065401 A1 | 3/2015  | Xu et al.      |
| 2011/0135805 A1  | 6/2011  | Doucet et al.       | 2015/0240337 A1 | 8/2015  | Sherman et al. |
| 2011/0135953 A1  | 6/2011  | Xu et al.           | 2015/0299838 A1 | 10/2015 | Doud et al.    |
| 2011/0136707 A1  | 6/2011  | Xu et al.           | 2016/0209391 A1 | 7/2016  | Zhang et al.   |
| 2011/0139465 A1  | 6/2011  | Tibbles et al.      | 2016/0258242 A1 | 9/2016  | Hayter et al.  |
| 2011/0147014 A1  | 6/2011  | Chen et al.         | 2017/0044675 A1 | 2/2017  | Xu et al.      |
| 2011/0186306 A1  | 8/2011  | Marya et al.        |                 |         |                |
| 2011/0214881 A1  | 9/2011  | Newton              |                 |         |                |
| 2011/0247833 A1  | 10/2011 | Todd et al.         |                 |         |                |
| 2011/0253387 A1  | 10/2011 | Ervin               |                 |         |                |
| 2011/0256356 A1  | 10/2011 | Tomantschger et al. |                 |         |                |
| 2011/0259610 A1  | 10/2011 | Shkurti et al.      |                 |         |                |
| 2011/0277987 A1  | 11/2011 | Frazier             |                 |         |                |
| 2011/0277989 A1  | 11/2011 | Frazier             |                 |         |                |
| 2011/0284232 A1  | 11/2011 | Huang               |                 |         |                |
| 2011/0284240 A1  | 11/2011 | Chen et al.         |                 |         |                |
| 2011/0284243 A1  | 11/2011 | Frazier             |                 |         |                |
| 2011/0300403 A1  | 12/2011 | Vecchio et al.      |                 |         |                |
| 2011/0314881 A1  | 12/2011 | Hatcher et al.      |                 |         |                |
| 2012/0046732 A1  | 2/2012  | Sillekens et al.    |                 |         |                |
| 2012/0067426 A1  | 3/2012  | Soni et al.         |                 |         |                |
| 2012/0090839 A1  | 4/2012  | Rudic               |                 |         |                |
| 2012/0103135 A1  | 5/2012  | Xu et al.           |                 |         |                |
| 2012/0107590 A1  | 5/2012  | Xu et al.           |                 |         |                |
| 2012/0118583 A1  | 5/2012  | Johnson et al.      |                 |         |                |
| 2012/0130470 A1  | 5/2012  | Agnew               |                 |         |                |
| 2012/0145378 A1  | 6/2012  | Frazier et al.      |                 |         |                |
| 2012/0145389 A1  | 6/2012  | Fitzpatrick, Jr.    |                 |         |                |
| 2012/0168152 A1  | 7/2012  | Casciaro et al.     |                 |         |                |
| 2012/0177905 A1  | 7/2012  | Seals et al.        |                 |         |                |
| 2012/0205120 A1  | 8/2012  | Howell              |                 |         |                |
| 2012/0205872 A1  | 8/2012  | Reinhardt et al.    |                 |         |                |
| 2012/0211239 A1  | 8/2012  | Kritzler et al.     |                 |         |                |
| 2012/0234546 A1  | 9/2012  | Xu et al.           |                 |         |                |
| 2012/0234547 A1  | 9/2012  | O'Malley et al.     |                 |         |                |
| 2012/0267101 A1  | 10/2012 | Cooke               |                 |         |                |
| 2012/0269673 A1  | 10/2012 | Koo et al.          |                 |         |                |
| 2012/0292053 A1  | 11/2012 | Xu et al.           |                 |         |                |
| 2012/0318513 A1  | 12/2012 | Mazyar et al.       |                 |         |                |
| 2013/0004847 A1  | 1/2013  | Kumar et al.        |                 |         |                |
| 2013/0008671 A1  | 1/2013  | Booth et al.        |                 |         |                |
| 2013/0025409 A1  | 1/2013  | Xu                  |                 |         |                |
| 2013/0029886 A1  | 1/2013  | Mazyar et al.       |                 |         |                |
| 2013/0032357 A1  | 2/2013  | Mazyar et al.       |                 |         |                |
| 2013/0048304 A1  | 2/2013  | Agrawal et al.      |                 |         |                |
| 2013/0048305 A1  | 2/2013  | Xu et al.           |                 |         |                |
| 2013/0052472 A1  | 2/2013  | Xu                  |                 |         |                |
| 2013/0081814 A1  | 4/2013  | Gaudette et al.     |                 |         |                |
| 2013/0084643 A1  | 4/2013  | Commarie et al.     |                 |         |                |
| 2013/0105159 A1  | 5/2013  | Alvarez             |                 |         |                |
| 2013/0126190 A1  | 5/2013  | Mazyar et al.       |                 |         |                |
| 2013/0131966 A1  | 5/2013  | Hirano              |                 |         |                |
| 2013/0133897 A1  | 5/2013  | Baihly et al.       |                 |         |                |
| 2013/0144290 A1  | 6/2013  | Schiffl et al.      |                 |         |                |
| 2013/0146144 A1  | 6/2013  | Joseph et al.       |                 |         |                |
| 2013/0146302 A1  | 6/2013  | Gaudette et al.     |                 |         |                |
| 2013/0167502 A1* | 7/2013  | Wilson .....        | B29C 70/025     |         |                |
|                  |         |                     | 57/210          |         |                |

|                 |         |                |
|-----------------|---------|----------------|
| 2014/0116711 A1 | 5/2014  | Tang et al.    |
| 2014/0186207 A1 | 7/2014  | Bae et al.     |
| 2014/0190705 A1 | 7/2014  | Fripp et al.   |
| 2014/0196899 A1 | 7/2014  | Jordan et al.  |
| 2014/0262327 A1 | 9/2014  | Xu et al.      |
| 2014/0360728 A1 | 12/2014 | Tashiro et al. |
| 2015/0060085 A1 | 3/2015  | Xu             |
| 2015/0065401 A1 | 3/2015  | Xu et al.      |
| 2015/0240337 A1 | 8/2015  | Sherman et al. |
| 2015/0299838 A1 | 10/2015 | Doud et al.    |
| 2016/0209391 A1 | 7/2016  | Zhang et al.   |
| 2016/0258242 A1 | 9/2016  | Hayter et al.  |
| 2017/0044675 A1 | 2/2017  | Xu et al.      |

### FOREIGN PATENT DOCUMENTS

|    |               |         |
|----|---------------|---------|
| CN | 1076968 A     | 10/1993 |
| CN | 1079234 A     | 12/1993 |
| CN | 1255879 A     | 6/2000  |
| CN | 2658384 Y     | 11/2004 |
| CN | 1668545 A     | 9/2005  |
| CN | 101050417 A   | 10/2007 |
| CN | 101351523 A   | 1/2009  |
| CN | 101454074 A   | 6/2009  |
| CN | 101457321 A   | 6/2009  |
| CN | 101605963     | 12/2009 |
| CN | 101720378 A   | 6/2010  |
| EP | 0033625 A1    | 8/1981  |
| EP | 1174385 A2    | 1/2002  |
| EP | 1412175 A1    | 4/2004  |
| EP | 1798301 A1    | 8/2006  |
| EP | 1857570 A2    | 11/2007 |
| FR | 2782096 A1    | 2/2000  |
| GB | 912956 A      | 12/1962 |
| GB | 1046330 A     | 10/1966 |
| GB | 1280833 A     | 7/1972  |
| GB | 1357065 A     | 6/1974  |
| JP | 61067770 A    | 4/1986  |
| JP | 754008 A      | 2/1995  |
| JP | 8232029 A     | 9/1996  |
| JP | 2000185725 A1 | 7/2000  |
| JP | 2002053902 A  | 2/2002  |
| JP | 2004225084 A  | 8/2004  |
| JP | 2004225765 A  | 8/2004  |
| JP | 2005076052 A  | 3/2005  |
| JP | 2010502840 A  | 1/2010  |
| KR | 950014350 B1  | 11/1995 |
| WO | 9909227 A1    | 2/1999  |
| WO | 9947726 A1    | 9/1999  |
| WO | 2004001087 A1 | 12/2003 |
| WO | 2004073889 A1 | 9/2004  |
| WO | 2005040068 A  | 5/2005  |
| WO | 2007044635 A  | 4/2007  |
| WO | 2007095376 A2 | 8/2007  |
| WO | 2008034042 A3 | 3/2008  |
| WO | 2008057045 A1 | 5/2008  |
| WO | 2008079485 A2 | 7/2008  |
| WO | 2008079777 A2 | 7/2008  |
| WO | 2009079745 A1 | 7/2009  |
| WO | 2010012184 A1 | 2/2010  |
| WO | 2010083826    | 7/2010  |
| WO | 2011071902 A2 | 6/2011  |
| WO | 2011071907 A2 | 6/2011  |
| WO | 2011071910 A2 | 6/2011  |
| WO | 2011130063 A3 | 2/2012  |
| WO | 2012015567 A2 | 2/2012  |
| WO | 2012149007 A2 | 11/2012 |
| WO | 2012174101 A2 | 12/2012 |
| WO | 2013053057 A1 | 4/2013  |
| WO | 2013078031 A1 | 5/2013  |
| WO | 2014121384 A1 | 8/2014  |
| WO | 2016085798    | 6/2016  |

### OTHER PUBLICATIONS

“Declaration of Karl T. Hartwig in Support of Petitioner Pursuant to 37 C.F.R. § 42.120”, executed on Nov. 21, 2016 in support of U.S. Pat. No. 9,101,978, 51 pages.

(56)

## References Cited

## OTHER PUBLICATIONS

- Adams, et al.; "Thermal stabilities of aromatic acids as geothermal tracers", *Geothermics*, vol. 21, No. 3, 1992, pp. 323-339.
- Aviles et al, "Degradable Alternative to Risky Mill-Out Operations in Plug and Perf"; SPE-173695-MS; Society of Petroleum Engineers; SPE/ICOTA Coiled Tubing & Well Intervention Conference & Exhibition; Mar. 24-25, 2015; 10 Pages.
- Ayman, et al.; "Effect of Consolidation and Extrusion Temperatures on Tensile Properties of Hot Extruded ZK61 Magnesium Alloy Gas Atomized Powders via Spark Plasma Sintering", *Transactions of JWRI*, vol. 38 (2009), No. 2, pp. 1-5.
- Baker Hughes Incorporated. IN-Tallic Disintegrating Frac Balls. Houston: Baker Hughes Incorporated, 2011. Accessed Mar. 6, 2015.
- Baker Hughes, "Multistage", Oct. 31, 2011, BakerHughes.com; accessed Mar. 6, 2015.
- Bin et al., "Advances in Fluidization CVD Technology", East China University of Chemical Technology, China Academic Journal Electronic Publishing House, vol. 13, No. 4, Nov. 1992, pp. 360-365, English Abstract on p. 366.
- Callister, Jr., William D., *Materials Science and Engineering an Introduction*, Seventh Edition, 2006, pp. 111, 627, and G7.
- Chuan-Jun et al., "Study on Corrosion Kinetics of Mg—Ni alloys", *Journal of Kunming University of Science and Technology*, vol. 34, No. 5, pp. 10-13, Oct. 2009.
- German, Randall M., *Powder Metallurgy Science*, Second Edition, 1994, 102 pages.
- Klar, Erhard, *ASM Handbook: International Metals Handbook—Powder Metallurgy*, vol. 7, 1997, pp. 14, 276, and 798.
- Lin et al., "Processing and Microstructure of Nano-Mo/A12O3 Composites from MOCVD and Fluidized Bed", *Nanostructured Materials*, Nov. 1999, vol. 11, No. 8, pp. 1361-1377.
- Petition for Inter Partes Review; Case No. IPR2017-00326; U.S. Pat. No. 9,101,978; Nov. 23, 2016; 46 pages.
- Petition for Inter Partes Review; Case No. IPR2017-00327; U.S. Pat. No. 8,573,295; Nov. 23, 2016; 53 pages.
- Reid, Gary Carl, "Literature evaluation of induced groundwater tracers, field tracer techniques, and hydrodynamic dispersion values in porous media", *Thesis in Geosciences (Masters)*, Texas Tech University, Aug. 1981, 109 pages.
- Rose, et al.; "The application of the polyaromatic sulfonates as tracers in geothermal reservoirs", *Geothermics* 30 (2001) pp. 617-640.
- Saravanan et al, "Mechanically Alloyed Carbon Nanotubes (CNT) Reinforced Nanocrystalline AA 4032: Synthesis and Characterization", *Journal of Minerals and Materials Characterization and Engineering*, vol. 9, No. 11 pp. 1027-1035 2010.
- Schaffer, James P. et al., *The Science and Design of Engineering Materials*, Second Edition, 1999, pp. 122, 123, 698, and 699.
- Shigematsu, et al., "Surface Treatment of AZ91D Magnesium Alloy by Aluminum diffusion Coating", *Journal of Materials Science Letters* 19, 2000, pp. 473-475.
- Singh, et al., "Extended Homogeneity Range of Intermetallic Phases in Mechanically Alloyed Mg—Al Alloys", Elsevier Sciences Ltd., *Intermetallics* 11, 2003, pp. 373-376.
- Spencer et al., "Fluidized Bed Polymer Particle ALD Process for Producing HDPE/Alumina Nanocomposites", The 12th International Conference on Fluidization—New Horizons in Fluidization Engineering, vol. RP4 (2007).
- Stanley, et al.; "An Introduction to Ground-Water Tracers", Department of Hydrology and Water Resources, University of Arizona, Mar. 1985, pp. 1-219.
- Tsipas et al. "Effect of High Energy Ball Milling on Titanium-Hydroxyapatite Powders" *Powder Metallurgy*, Maney Publishing, London, GB, vol. 46, No. 1, Mar. 2003 (Mar. 2003), pp. 73-77.
- Xie, Guoqiang et al., "TEM Observation of Interfaces between Particles in Al—Mg Alloy Powder Compacts Prepared by Pulse Electric Current Sintering", *Materials Transactions*, 2002, pp. 2177-2180, vol. 43—No. 9.
- Zemel, "Tracers in the Oil Field", University of Texas at Austin, Center for Petroleum and Geosystems, Jan. 1995, Chapters 1, 2, 3, 7.
- "Optisleeve Sliding Sleeve", [online]; [retrieved on Jun. 25, 2010]; retrieved from the Internet [weatherfordcorp/WFT033159.pdf](http://weatherford.com/weatherford/groups/.../weatherfordcorp/WFT033159.pdf).
- Baker Hughes, "Flow Control Systems," [online]; [retrieved on May 20, 2010]; retrieved from the Internet <http://www.bakerhughes.com/products-and-services/completions-and-productions/well-completions/packers-and-flow-control/flow-control-systems>.
- Bououdina, et al., "Comparative Study of Mechanical Alloying of (Mg-Al) and (Mg+Al+Ni) Mixtures for Hydrogen Storage", *J. Alloys, Compds*, 2002, 336, 222-231.
- Carrejo, et al., "Improving Flow Assurance in Multi-Zone Fracturing Treatments in Hydrocarbon Reservoirs with High Strength Corrodible Tripping Balls"; Society of Petroleum Engineers; SPE Paper No. 151613; Apr. 16, 2012; 5 pages.
- Coronado, "Development of an Internal Coiled Tubing Connector Utilizing Permanent Packer Technology"; Society of Petroleum Engineers, SPE Paper No. 46036; Apr. 15, 1998; 10 pages.
- Garfield, New One-Trip Sand-Control Completion System that Eliminates Formation Damage Resulting From conventional Perforating and Gravel-Pack Operations:, SPE Annual Technical Conference and Exhibition, Oct. 9-12, 2005.
- Gray, et al., "Protective Coatings on Magnesium and Its Alloys—a Critical Review", *Journal of Alloys and Compounds* 336 (2002), pp. 88-113.
- Hsiao, et al., "Anodization of AZ91D Magnesium Alloy in Silicate-Containing Electrolytes"; *Surface & Coatings Technology*; 199; pp. 127-134; (2005).
- Hsiao, et al., "Characterization of Anodic Films Formed on AZ91D Magnesium Alloy"; *Surface & Coatings Technology*; 190; pp. 299-308; (2005).
- Huo et al.; "Corrosion of AZ91D Magnesium Alloy with a Chemical Conversion Coating and Electroless Nickel Layer"; *Corrosion Science*; 46; pp. 1467-1477; (2004).
- Kuzumaki, et al.; "Mechanical Characteristics and Preparation of Carbon Nanotube Fiber-Reinforced Ti Composite", *Advanced Engineering Materials*, 2000, 2, No. 7.
- Liu, et al., "Calculated Phase Diagrams and the Corrosion of Die-Cast Mg—Al Alloys", *Corrosion Science*, 2009, 51, 606-619.
- Lunder et al.; "The Role of Mg17Al12 Phase in the Corrosion of Mg Alloy AZ91", *Corrosion*; 45(9); pp. 741-748; (1989).
- Majumdar, et al., "Laser Surface Engineering of a Magnesium Alloy with Al + Al2O3", *Surface and Coatings Technology* 179 (2004) pp. 297-305.
- Murray, "Binary Alloy Phase Diagrams" *Int. Met. Rev.*, 30(5) 1985 vol. 1, pp. 103-187.
- Nie, "Patents of Methods to Prepare Intermetallic Matrix Composites: A Review", *Recent Patents on Materials Science* 2008, vol. 1, pp. 232-240.
- Saravanan et al., "Mechanically Alloyed Carbon Nanotubes (CNT) Reinforced Nanocrystalline AA 4032: Synthesis and Characterization," *Journal of Minerals & Materials Characterization & Engineering*, vol. 9, No. 11, pp. 1027-1035, 2010.
- Shaw, "Benefits and Application of a Surface-Controlled Sliding Sleeve for Fracturing Operations"; Society of Petroleum Engineers, SPE Paper No. 147546; Oct. 30, 2011; 8 pages.
- Song, "Recent Progress in Corrosion and Protection of Magnesium Alloys"; *Advanced Engineering Materials*; 7(7); pp. 563-586; (2005).
- Song, et al.; "A Possible Biodegradable Magnesium Implant Material," *Advanced Engineering Materials*, vol. 9, Issue 4, Apr. 2007, pp. 298-302.
- Song, et al.; "Corrosion Behaviour of AZ21, AZ501 and AZ91 in Sodium Chloride"; *Corrosion Science*; 40(10); pp. 1769-1791; (1998).
- Triolo et al., "Resolving the Completion Engineer's Dilemma: Permanent or Retrievable Packer?", Society of Petroleum Engineers, SPE Paper No. 76711; May 20, 2002; 16 pages.
- Vernon Constien et al., "Development of Reactive Coatings to Protect Sand-Control Screens", SPE 112494, Copyright 2008, Soci-

(56)

## References Cited

## OTHER PUBLICATIONS

- ety of Petroleum Engineers, Presented at the 2008 SPE International Symposium and Exhibition on Formation Damage Control.
- Walters, et al.; "A Study of Jets from Unsintered-Powder Metal Lined Nonprecision Small-Caliber Shaped Charges", Army Research Laboratory, Aberdeen Proving Ground, MD 21005-5066; Feb. 2001.
- Wang, et al., "Contact-Damage-Resistant Ceramic/Single-Wall Carbon Nanotubes and Ceramic/Graphite Composites" *Nature Materials*, vol. 3, Aug. 2004, pp. 539-544.
- Watanabe, et al., "Superplastic Deformation Mechanism in Powder Metallurgy Magnesium Alloys and Composites", *Acta mater.* 49 (2001) pp. 2027-2037.
- Watarai, Trend of research and development for magnesium alloys-reducing the weight of structural materials in motor vehicles, (2006) Science and technology trends, Quaterly review No. 18, 84-97.
- Welch, et al., "Nonelastomeric Sliding Sleeve Maintains Long Term Integrity in HP/HT Application: Case Histories" [Abstract Only], SPE Eastern Regional Meeting, Oct. 23-25, 1996, Columbus, Ohio.
- Xu, et al., "Nanostructured Material-Based Completion Tools Enhance Well Productivity"; International Petroleum Technology Conference; Conference Paper IPTC 16538; International Petroleum Technology Conference 2013; 4 pages.
- Zhan, et al., "Single-wall carbon nanotubes as attractive toughening agents in alumina-based nanocomposites" *Nature Materials*, vol. 2, Jan. 2003, pp. 38-42.
- Zhang, et al.; "Formation of metal nanowires on suspended single-walled carbon nanotubes" *Applied Physics Letter*, vol. 77, No. 19 (2000), pp. 3015-3017.
- Zhang, et al.; "Study on the Environmentally Friendly Anodizing of AZ91D Magnesium Alloy"; *Surface and Coatings Technology*: 161; pp. 36-43; (2002).
- Zhu, et al., "The process of coating on ultrafine particles by surface hydrolysis reaction in a fluidized bed reactor", *Surface and Coatings Technology* 135 (2000) 14-17.
- "Baker Hughes Refines Expandable Tubular Technology with Abaqus and Isight", *Simulia Realistic Simulation News*, Jan./Feb. 2011, pp. 12-13.
- "Reactivity series", Wikipedia, [http://en.wikipedia.org/w/index.php?title=Reactivity\\_series&printable=yes](http://en.wikipedia.org/w/index.php?title=Reactivity_series&printable=yes) downloaded on May 18, 2014. 8 pages.
- Bakshi et al., "Carbon nanotube reinforced metal matrix composites—a review," *International Materials Reviews*; 2010, pp. 41-64, vol. 55, No. 1.
- Birbilis, et al., "Exploring Corrosion Protection of Mg Via Ionic Liquid Pretreatment", *Surface & Coatings Technology*; 201, pp. 4496-4504, (2007).
- Feng, et al., "Electroless Plating of Carbon Nanotubes with Silver" *Journal of Materials Science*, 39, (2004) pp. 3241-3243.
- Lee, et al., "Effects of Ni addition on hydrogen storage properties of Mg17Al12 alloy", *Materials Chemistry and Physics*, 2011, 126, pp. 319-324.
- Li, et al., "Investigation of aluminium-based nanocomposites with ultra-high strength", *Materials Science and Engineering A*, 527, pp. 305-316, (2009).
- Liu, et al.; "Electroless Nickel Plating on AZ91 Mg Alloy Substrate"; *Surface & Coatings Technology*; 200; pp. 5087-5093; (2006).
- Mathis, "Sand Management: A Review of Approaches and Concerns", Society of Petroleum Engineers, SPE Paper No. 82240, SPE European Formation Damage Conference, The Hague, The Netherlands, May 13-14, 2003.
- Pardo, et al.; "Corrosion Behaviour of Magnesium/Aluminium Alloys in 3.5 wt% NaCl"; *Corrosion Science*; 50; pp. 823-834; (2008).
- Quik Drill Composite Frac Plug; Baker Hughes, Baker Oil Tools; Copyright 2002; 3 pages.
- Shi, et al.; "Influence of the Beta Phase on the Corrosion Performance of Anodised Coatings on Magnesium-Aluminium Alloys"; *Corrosion Science*; 47; pp. 2760-2777; (2005).
- Shimizu, et al., "Multi-walled carbon nanotube-reinforced magnesium alloy composites", *Scripta Materialia*, vol. 58, Issue 4, Feb. 2008, pp. 267-270.
- Shumbera, et al. "Improved Water Injector Performance in a Gulf of Mexico Deepwater Development Using an Openhole Frac Pack Completion and Downhole Filter System: Case History." SPE Annual Technical Conference and Exhibition, Oct. 5-8, 2003.
- Song, et al.; "Corrosion Mechanisms of Magnesium Alloys"; *Advanced Engineering Materials*; 1(1); pp. 11-33; (1999).
- Song, et al.; "Influence of Microstructure on the Corrosion of Diecast AZ91D"; *Corrosion Science*; 41; pp. 249-273; (1999).
- Song, et al.; "Understanding Magnesium Corrosion"; *Advanced Engineering Materials*; 5; No. 12; pp. 837-858; (2003).
- Sun, et al.; "Colloidal Processing of Carbon Nanotube/Alumina Composites" *Chem. Mater.* 2002, 14, pp. 5169-5172.
- Vickery, et al.; "New One-Trip Multi-Zone Frac Pack System with Positive Positioning." European Petroleum Conference, Oct. 29-31, 2002, Aberdeen, UK. [Abstract Only].
- Zeng, et al. "Progress and Challenge for Magnesium Alloys as Biomaterials," *Advanced Engineering Materials*, vol. 10, Issue 8, Aug. 2008, pp. B3-B14.
- Zhang, et al.; "High Strength Nanostructured Materials and Their Oil Field Applications"; Society of Petroleum Engineers; Conference Paper SPE 157092; SPE International Oilfield Nanotechnology Conference, 2012; 6 pages.
- Zhang, et al.; "Metal Coating on Suspended Carbon Nanotubes and its Implication to Metal-Tube Interaction", *Chemical Physics Letters* 331 (2000) 35-41.
- "Sliding Sleeve", Omega Completion Technology Ltd, Sep. 29, 2009, retrieved on: [www.omega-completion.com](http://www.omega-completion.com).
- Ambat, et al., "Electroless Nickel-Plating on AZ91D Magnesium Alloy: Effect of Substrate Microstructure and Plating Parameters"; *Surface and Coatings Technology*; 179; pp. 124-134; (2004).
- Baker Oil Tools, "Baker Oil Tools Introduces Revolutionary Sand Control Completion Technology," May 2, 2005.
- Baker Oil Tools, "Z-Seal Metal-to-Metal Expandable Sealing Device Uses Expanding Metal in Place of Elastomers," Nov. 6, 2006.
- Bastow, et al., "Clustering and formation of nano-precipitates in dilute aluminum and magnesium alloys", *Materials Science and Engineering*, 2003, C23, 757-762.
- Bercegeay, et al., "A One-Trip Gravel Packing System"; Society of Petroleum Engineers, Offshore Technology Conference, SPE Paper No. 4771; Feb. 7-8, 1974.
- Bybee, "One-Trip Completion System Eliminates Perforations," *Completions Today*, Sep. 2007, pp. 52-53.
- Chang, et al., "Electrodeposition of Aluminum on Magnesium Alloy in Aluminum Chloride (AlCl<sub>3</sub>)-1-ethyl-3-methylimidazolium chloride (EMIC) Ionic Liquid and Its Corrosion Behavior"; *Electrochemistry Communications*; 9; pp. 1602-1606; (2007).
- Christoglou, et al., "Deposition of Aluminum on Magnesium by a CVD Process", *Surface and Coatings Technology* 184 (2004) 149-155.
- Constantine, "Selective Production of Horizontal Openhole Completions Using ECP and Sliding Sleeve Technology." SPE Rocky Mountain Regional Meeting, May 15-18, 1999, Gillette, Wyoming. [Abstract Only].
- Curtin, et al., "CNT-reinforced ceramics and metals," *Materials Today*, 2004, vol. 7, pp. 44-49.
- Flahaut, et al., "Carbon Nanotube-Metal-Oxide Nanocomposites: Microstructure, Electrical Conductivity and Properties" *Acta amter.* 48 (2000), pp. 3803-3812.
- Forsyth, et al.; "An Ionic Liquid Surface Treatment for Corrosion Protection of Magnesium Alloy AZ31"; *Electrochim. Solid-State Lett.* 2006 vol. 9, Issue 11, B52-B55/ 9(11); Abstract only; 1 page.
- Galanty, et al. "Consolidation of metal powders during the extrusion process," *Journal of Materials Processing Technology* (2002), pp. 491-496.
- Garfield, "Formation Damage Control Utilizing Composite-Bridge-Plug Technology for Monobore, Multizone Stimulation Operations," SPE 70004, 2001, Society of Petroleum Engineers Inc., This paper was prepared for presentation at the SPE Per.

(56)

**References Cited****OTHER PUBLICATIONS**

Garfield, et al., "Maxmizing Inflow Performance in Soft Sand Completions Using New One-trip Sand Control Liner Completion Technology", SPE European Formation Damage Conference, May 25-27, 2005.

Goh, et al., "Development of novel carbon nanotube reinforced magnesium nanocomposites using the powder metallurgy technique", Nanotechnology 17 (2006) 7-12.

Han, et al., "Mechanical Properties of Nanostructured Materials", Rev. Adv. Mater. Sci. 9(2005) 1-16.

Hermawan, et al., "Iron-manganese: new class of metallic degradable biomaterials prepared by powder metallurgy", Powder Metallurgy, vol. 51, No. 1, (2008), pp. 38-45.

Hjortsam, et al. "Can we achieve ultra-low resistivity in carbon nanotube-based metal composites," Applied Physics A (2004), vol. 78, Issue 8, pp. 1175-1179.

Hsiao, et al., "Baking Treatment Effect on Materials Characteristics and Electrochemical Behavior of anodic Film Formed on AZ91D Magnesium Alloy"; Corrosion Science; 49; pp. 781-793; (2007).

Hsiao, et al., "Effect of Heat Treatment on Anodization and Electrochemical Behavior of AZ91D Magnesium Alloy"; J. Mater. Res.; 20(10); pp. 2763-2771;(2005).

Lavernia, et al., "Cryomilled Nanostructured Materials: Processing and Properties", Materials Science and Engineering A, 493, (2008) pp. 207-214.

Li, "Design of Abrasive Water Jet Perforation and Hydraulic Fracturing Tool," Oil Field Equipment, Mar. 2011.

Maisano, "Cryomilling of Aluminum-Based and Magnesium-Based Metal Powders", Thesis, Virginia Tech, Jan. 13, 2006.

Seyni, et al., "On the interest of using degradable fillers in co-ground composite materials", Powder Technology 190, (2009) pp. 176-184.

Vahlas, et al., "Principles and Applications of CVD Powder Technology", Materials Science and Engineering R 53 (2006) pp. 1-72.

\* cited by examiner



FIG. 1



FIG. 2



FIG. 3



FIG. 4

## 1

**METHODS OF MANUFACTURING  
DEGRADABLE TOOLS USING A GALVANIC  
CARRIER AND TOOLS MANUFACTURED  
THEREOF**

**BACKGROUND**

The disclosure is directed to methods of manufacturing degradable tools, and in particular to methods of manufacturing degradable tools using a galvanic carrier. The disclosure also relates to the tools manufactured by the methods.

Oil and natural gas, or carbon dioxide sequestration wells often utilize wellbore components or tools that, due to their function, are only required to have limited service lives that are considerably less than the service life of the well. After a component or tool service function is complete, it must be removed or disposed of in order to recover the original size of the fluid pathway for use, including hydrocarbon production, CO<sub>2</sub> sequestration, etc.

To facilitate removal, such tools or components may be formed of a corrodible material so that they need not be physically removed by, for example, a mechanical operation, but may instead corrode or degrade under downhole conditions.

Despite all the advances, the art is still receptive to alternative methods of manufacturing degradable tools, in particular methods that are effective to manufacture tools having uniform degradation rates.

**BRIEF DESCRIPTION**

In an embodiment, a method of manufacturing an article is provided. The method comprises forming a mixture comprising composite particles dispersed in a metallic matrix material; the composite particles comprising a carrier and a disintegration agent coated on the carrier or embedded in the carrier, or a combination thereof and having a density that is about 0.2 to about 2.5 equivalents to that of the metallic matrix material when measured under the same testing conditions; and molding or casting the mixture to form a degradable article; wherein the disintegration agent forms a plurality of galvanic cells with the metallic matrix material, or the carrier, or a combination thereof, in the degradable article.

Also disclosed is a degradable article produced by the method.

In another embodiment, a degradable article is provided. The article comprises: a metallic matrix comprising a plurality of grains formed from a metallic matrix material, a carrier, or a combination thereof; and a disintegration agent disposed on grain boundaries of the grains formed from the metallic matrix material, the carrier, or a combination thereof; the disintegration agent comprising particles having an aspect ratio greater than about 2; wherein the disintegration agent form a plurality of galvanic cells in the article with the metallic matrix material, the carrier, or a combination thereof.

**BRIEF DESCRIPTION OF THE DRAWINGS**

Referring now to the drawings wherein like elements are numbered alike in the several Figures:

FIG. 1 illustrates a composite particle comprising a carrier coated with a disintegration agent;

FIG. 2 illustrates a composite particle comprising a carrier and a coating; where the coating comprising a disintegration agent;

## 2

FIG. 3 illustrates a composite particle comprising a carrier with a disintegration agent partially or fully embedded in the carrier; and

FIG. 4 illustrates a composite particle comprising a carrier with a disintegration agent embedded in the carrier as well as coated on the surface of the carrier.

**DETAILED DESCRIPTION**

10 Metals and metal alloys having a high activity on the saltwater galvanic series, such as a magnesium alloy, can be used as a matrix material to form degradable articles. A disintegration agent can be added to the matrix material to adjust the degradation rate. One method of forming the 15 degradable article includes molding a solid-liquid mixture comprising solid disintegration agent particles dispersed in a molten matrix material. To form articles having controlled degradation rate, it is desirable to form a homogeneous solid liquid mixture. However, certain disintegration agents are 20 much heavier than the matrix materials. Thus in the solid liquid mixture, these heavy disintegration agents have a tendency to precipitate in the light molten matrix material, which makes it challenging to achieve uniform distribution of the disintegration agents.

25 The inventors hereof have found that degradable articles having a controlled and uniform degradation rate can be made from a matrix material and composite particles comprising a carrier and a disintegration agent. In particular, the materials for the carrier and the disintegration agent as well 30 as the amounts of the carrier and the disintegration agent are selected such that the composite particles formed thereof have a density that is about 0.5 to about 1.5 equivalents to that of the metallic matrix material when measured under the same testing conditions. The disintegration agent is coated 35 on the carrier or embedded in the carrier, or a combination thereof. When such composite particles are mixed with matrix materials, the composite particles can be uniformly distributed in the molten matrix material. Under the process 40 conditions, the carrier can partially or completely melt releasing the disintegration agent. In the instance where the disintegration agent is coated on the carrier, upon the melting of the carrier (core), under agitation forces, the coating breaks into particles. Because the coating can have a thickness of only a few nanometers, the disintegration particles 45 formed upon melting of the carrier can have a high aspect ratio. The high aspect ratio facilitates the maintenance of uniform distribution of the disintegration agent. Upon cooling, the uniformly distributed and released disintegration agent can be “frozen” in this place. Without wishing to be 50 bound by theory, it is believed that the disintegration agent can then act as nucleation site for solidification of molten matrix material. As a further advantageous feature, the carrier forms galvanic cells with the disintegration agent allowing further control over the degradation rate of the 55 article.

The matrix material comprises one or more of the following: a magnesium-based alloy; an aluminum-based alloy; or a zinc-based alloy. As used herein, the term “metal-based alloy” means a metal alloy wherein the weight 60 percentage of the specified metal in the alloy is greater than the weight percentage of any other component of the alloy, based on the total weight of the alloy.

Magnesium-based alloys suitable for use include alloys of magnesium with aluminum (Al), cadmium (Cd), calcium (Ca), cobalt (Co), copper (Cu), iron (Fe), manganese (Mn), nickel (Ni), silicon (Si), silver (Ag), strontium (Sr), thorium (Th), tungsten (W), zinc (Zn), zirconium (Zr), or a combi-

nation comprising at least one of these elements. Alloying or trace elements can be included in varying amounts to adjust the corrosion rate of the magnesium. Exemplary commercial magnesium-based alloys which include different combinations of the above alloying elements to achieve different degrees of corrosion resistance include but are not limited to, for example, those alloyed with aluminum, strontium, and manganese such as AJ62, AJ50x, AJ51x, and AJ52x alloys, and those alloyed with aluminum, zinc, and manganese such as AZ91A-E alloys. Other exemplary magnesium-based alloys include MgZrZn, MgAlZn, AlCuZnMn, and AlMg-ZnSiMn.

Aluminum-based alloys include all alloys that have aluminum as an alloy constituent. Exemplary aluminum alloys include Al—Cu alloy, Al—Mn alloy, Al—Si alloy, Al—Mg alloy, Al—Mg—Si alloy, Al—Zn alloy, Al—Li alloy, Al—Cu—Mg—X alloy, Al—Zn—Mg—Cu—X, where X represents alloying elements including Zn, Mn, Si, Cr, Fe, Ni, Ti, V, Cu, Pb, Bi, and Zr.

Zinc-based alloys include alloys of zinc with Al, Cu, Mg, Pb, Cd, Sn, Fe, Ni, Si, or a combination of the above elements. In a specific embodiment, the metallic matrix material is a magnesium alloy.

The composite particles comprise a carrier and a disintegration agent, wherein the disintegration agent is coated on the surface of the carrier, embed in the carrier, or a combination thereof. FIGS. 1-4 illustrate composite particles according to various embodiments of the disclosure. In FIG. 1, the composite particle comprises carrier 11 coated with disintegration particles 10. In FIG. 2, the disintegration agent forms a coating 20 on the surface of the carrier 21. In FIG. 3, the composite particle comprises carrier 31, disintegration particles 32 that are fully embedded in carrier 31 and disintegration particle 33 that are partially embedded in carrier 31. In FIG. 4, the composite particle comprises carrier 41, disintegration particles 42 that are fully embedded in carrier 41, disintegration particles 43 that are partially embedded in carrier 41 and disintegration particles 42 that are not embedded but disposed on the surface of carrier 41.

The disintegration agents have a higher melting point as compared to the metallic matrix material so that the metallic matrix material can be selectively melted during the manufacturing process. In an embodiment, the disintegration agents also have a higher melting point than the carrier so that the carrier is at last partially melted during the process conditions. Exemplary disintegration agents include one or more of the following: a metal; an oxide of the metal; a nitride of the metal; or a cermet of the metal; wherein the metal is one or more of the following: W; Co; Cu; Ni; or Fe. The disintegration agents can be in the form of a coating or particles embedded or disposed on a surface of the carrier. In the instance where the disintegration agents are particles, the particles can have an average particle size of about 50 nanometers to about 250 microns or about 1 to about 25 microns.

The carrier comprises one or more of the following: a magnesium-based alloy; an aluminum-based alloy; or a zinc-based alloy. The carrier can be same or different from the matrix material. The carrier comprises particles having an average particle size of about 1 micron to about 10 millimeters, or 50 microns to about 1 millimeter.

The composite particles have a density of about 0.2 to about 2.5 equivalents to that of the matrix material when tested under the same testing conditions. In another embodiment, the composite particles have a density of about 0.5 to about 1.5 equivalents to that of the matrix material when measured under the same testing conditions. The amount of

the disintegration agent in the composite particles is about 0.01 wt % to about 50 wt %, or about 1 wt % to about 10 wt %, based on the total weight of the composite particles.

Methods of making the composite particles are not particularly limited. Suitable methods include physical vapor deposition, chemical deposition, milling, mechanical mixing or the like. Physical vapor deposition and vapor deposition are particularly suitable for making composite particles comprising disintegration agent coated on the carrier.

The disintegration agent, which has a lower reactivity relative to the metallic matrix material and the carrier, acts as a cathode, whereas the metallic matrix and the carrier, which are more reactive than the disintegration agents, are anodic relative to the disintegration agents. A galvanic discharge cycle (e.g., corrosion) occurs between the relatively anodic and relatively cathodic materials in the presence of an electrolyte. By adjusting the compositions of the metallic matrix material, the carrier, and the disintegration agent and the amounts of the disintegration agents relative to the sum of the weight of the metallic matrix and the carrier, the corrosion rate of the degradable article is adjusted.

The composite particles can be present in an amount of about 0.1 wt % to about 50 wt % or 0.1 wt % to about 20 wt % based on the total weight of the mixture comprising the composite particles and metallic matrix material. The amount of the disintegration agents can vary depending on the specific materials used and desired corrosion rate. In an embodiment, the liquid-solid mixture comprises 0.001 to 10 wt %, or 0.05 to 8 wt %, or 0.1 to 6 wt % of the disintegration agents, based on the total weight of the mixture comprising the composite particles and the metallic matrix material.

One way to form the liquid-solid mixture is to mix the metallic matrix material in a solid form with the composite particles to provide a blend; and heating the blend optionally under agitation to selectively melt the metallic matrix material. Alternatively, the liquid solid mixture is made by heating the metallic matrix material in a solid form to provide a molten metallic matrix material; and introducing the composite particles to the molten matrix material under agitation. Heating the blend and heating the metallic matrix material can be conducted at a temperature above the melting point of the metallic matrix material. The carrier can be at least partially melted. In an embodiment, the heating is to a temperature of about 450° C. to about 850° C. The heating can be conducted at atmospheric pressure in the presence or absence of an inert atmosphere. In another embodiment, less than about 10 wt %, less than about 5 wt %, less than about 2 wt %, or less than about 1 wt % of the disintegration agents dissolve under the process conditions.

Optionally an agitation force is applied to the metallic matrix material and the composite particles during the mixing and heating. The agitation force can be generated by mechanical means, electromagnetic means, acoustic means, or a combination comprising at least one of the foregoing. For example, the metallic matrix material and the composite particles can be mechanically stirred in a crucible or a furnace. A magnetic field can also be applied to the metallic matrix material and the composite particles. By randomly changing the field direction, the magnitude, and the frequency of the field, an agitation force is generated. Alternatively or in addition to mechanical and electromagnetic forces, an acoustic generator such as a megasonic energy source imparts wave energy to the metallic matrix material and the disintegration agents and thus agitating them during the mixing.

The homogeneous liquid-solid mixture can be molded or casted. The casting method is not limited and includes die casting. To mold the liquid-solid mixture, the mixture is first disposed in a mold. The method of disposing is not particularly limited. For example, the homogeneous liquid-solid mixture can be poured into the mold, pushed into the mold under a superatmospheric pressure, or drawn to the mold under a subatmospheric pressure.

The molding can be a pressure molding or a vacuum molding. In an embodiment the molding is conducted at a pressure of about 500 psi to about 30,000 psi or about 1000 psi to about 5000 psi. The pressure can be a superatmospheric pressure or a subatmospheric pressure. In an embodiment, the mold is not heated. In another embodiment, the mold is heated to a temperature of about 90° C. to about 450° C. or about 150° C. to about 350° C. Optionally during the molding, an agitation force is applied to the mixture by mechanical means, electromagnetic means, acoustic means, or a combination comprising at least one of the foregoing.

The mold product is allowed to cool down to room temperature when the mold is still under pressure. In the instance where the molded product is subjected to a subsequent extrusion operation, the molded product can be cooled to a temperature above the room temperature. An agitation force is optionally applied to the molded product during the cooling process. The cooled article can be machined and used as is.

For applications requiring higher strength, the molded article is further extruded. During extrusion, the pores inside the molded product are fully closed to provide a condensed article having high tensile strength, high shear strength, and high compression strength. In addition, the extruded product dissolves more uniformly. The extrusion temperature is about 250° C. to about 450° C. or about 320° C. to about 420° C.

If necessary, the obtained articles can be further machined or shaped to form a bar, block, tubular, cylindrical billet, or toroid. Machining includes cutting, sawing, ablating, milling, facing, lathe, boring, and the like using, for example, a miller, saw, lathe, router, electric discharge machine, and the like.

The degradable article has a microstructure comprising a plurality of grains formed from the disintegration agent with the metallic matrix material, the carrier, or a combination of the metallic matrix material and the carrier. The grains have an average size of about 5 to about 300 microns. In an embodiment, the disintegration agents are disposed only on the grain boundaries. In another embodiment, the disintegration agents are disposed both on the grain boundaries and inside the grains.

When the composite particles comprise a carrier and a coating of the disintegration agent formed by methods such as chemical vapor deposition, the coating can have a thickness of 50 nanometers to 200 microns. During heating and/or mixing, the carrier at least partially melts. The unsupported coating breaks upon agitation into particles having a high aspect ratio. In an embodiment, the disintegration agent in the degradable article comprises particles having an aspect ratio greater than about 2, greater than about 4, or greater than about 6, or greater than about 10.

The degradable article thus has micron-sized or nanosized galvanic cells where the metallic matrix material and/or the carrier are the anode and the disintegration agents are cathode. The degradable article has uniform dissolution rate. In an embodiment, the degradable article has a corrosion rate of about 1 to about 300 mg/cm<sup>2</sup>/hour, specifically

about 10 to about 200 mg/cm<sup>2</sup>/hour using aqueous 3 wt % KCl solution at 200° F. (93° C.).

Articles formed from the method disclosed herein are not particularly limited. Articles formed from the method disclosed herein are not particularly limited. Exemplary tools include flappers, hold down dogs and springs, screen protectors, seal bore protectors, electric submersible pump space out subs, full bore guns, chemical encapsulations, slips, dogs, springs and collet restraints, liner setting sleeves, timing actuation devices, emergency grapple release, chemical encapsulation containers, screen protectors, beaded screen protectors, whipstock lugs, whipstock coatings, pins, set screws, emergency release tools, gas generators, mandrels, release mechanisms, staging collars, C-rings, components of perforating gun systems, disintegrable whipstock for casing exit tools, shear pins, dissolvable body locking rings, mud motor stators, progressive cavity pump stators, or shear screws.

20 The article can be a downhole tool. In an embodiment, the tool is a single component. In another embodiment the tool inhibits flow. In yet another embodiment, the tool is pumpable within a subterranean environment.

25 Pumpable tools include plugs, direct connect plugs, bridge plugs, wiper plugs, frac plugs, components of frac plugs, drill in sand control beaded screen plugs, inflow control device plugs, polymeric plugs, disappearing wiper plugs, cementing plugs, balls, diverter balls, shifting and setting balls, swabbing element protectors, buoyant recorders, pumpable collets, float shoes, or darts.

30 The tools that inhibit flow include seals, high pressure beaded frac screen plugs, screen basepipe plugs, coatings for balls and seats, compression packing elements, expandable packing elements, O-rings, attached seals, bullet seals, sub-surface safety valve seals, sub-surface safety valve flapper seal, dynamic seals, V-rings, back up rings, drill bit seals, liner port plugs, atmospheric discs, atmospheric chamber discs, debris barriers, drill in stim liner plugs, inflow control device plugs, flappers, seats, ball seats, direct connect disks, 35 drill-in linear disks, gas lift valve plug, fluid loss control flappers, electric submersible pump seals, shear out plugs, flapper valves, gaslift valves, or sleeves.

40 Methods to degrade an article comprises: exposing the polymer composition or the article to a fluid at a temperature of about 25° C. to about 300° C., about 65° C. to about 250° C., or about 65° C. to about 150° C. or about 175° C. to about 250° C. The pressure can be about 100 psi to about 15,000 psi.

45 The fluid can comprises water, brine, or a combination comprising at least one of the foregoing. The brine can include NaCl, KCl, NaBr, MgCl<sub>2</sub>, CaCl<sub>2</sub>, CaBr<sub>2</sub>, ZnBr<sub>2</sub>, NH<sub>4</sub>Cl, sodium formate, cesium formate, and the like.

50 Further included in this disclosure are the following specific embodiments, which do not necessarily limit the 55 claims.

#### Embodiment 1

A method of manufacturing a degradable article, the method comprising:

50 forming a mixture comprising composite particles dispersed in a metallic matrix material; the composite particles comprising a carrier and a disintegration agent coated on the carrier or embedded in the carrier, or a combination thereof and having a density that is about 0.2 to about 2.5 equivalents to that of the metallic matrix material when measured under the same testing conditions; and

molding or casting the mixture to form a degradable article;

wherein the disintegration agent forms a plurality of galvanic cells with the metallic matrix material, with the carrier, or with a combination of the metallic matrix material and the carrier, in the degradable article.

## Embodiment 2

The method of Embodiment 1 wherein the composite particles have a density that is about 0.5 to about 1.5 equivalents to that of the metallic matrix material when measured under the same testing conditions.

## Embodiment 3

The method of Embodiment 1 or Embodiment 2, further comprising forming the composite particles by one or more of the following: physical vapor deposition; chemical vapor deposition; milling; or mechanical mixing.

## Embodiment 4

The method of any one of Embodiments 1 to 3, wherein forming a mixture comprising composite particles dispersed in a metallic matrix material comprises:

mixing the metallic matrix material in a solid form with the composite particles to provide a blend; and

heating the blend to a temperature to selectively melt the metallic matrix material.

## Embodiment 5

The method of Embodiment 4, wherein the carrier is at least partially melted at the temperature.

## Embodiment 6

The method of any one of Embodiments 1 to 3, wherein forming a mixture comprising composite particles dispersed in a metallic matrix material comprises:

heating the metallic matrix material in a solid form to provide a molten metallic matrix material; and

introducing the composite particles to the molten matrix material.

## Embodiment 7

The method of Embodiment 6, wherein heating the metallic matrix material is to a temperature of about 450° C. to about 850° C.

## Embodiment 8

The method of any one of Embodiments 1 to 7, wherein molding the mixture comprises pressure molding or vacuum molding.

## Embodiment 9

The method of any one of Embodiments 1 to 8, wherein molding the mixture comprises applying a superatmospheric pressure of about 500 psi to about 30,000 psi to the mixture.

## Embodiment 10

The method of any one of Embodiments 1 to 9, further comprising extruding the molded article.

## Embodiment 11

The method of any one of Embodiments 1 to 10, wherein the carrier comprises one or more of the following: a magnesium-based alloy; an aluminum-based alloy; or a zinc-based alloy.

## Embodiment 12

The method of any one of Embodiments 1 to 11, wherein the carrier comprises particles have an average particle size of about 1 micron to about 10 millimeters.

## Embodiment 13

The method of any one of Embodiments 1 to 12, wherein the disintegration agent comprises one or more of the following: a metal; an oxide of the metal; a nitride of the metal; or a cermet of the metal; wherein the metal is one or more of the following: W; Co; Cu; Ni; or Fe.

## Embodiment 14

The method of any one of Embodiments 1 to 13, wherein the disintegration agent comprises particles having an average particle size of about 200 nanometers to about 10 microns.

## Embodiment 15

The method of any one of Embodiments 1 to 14, wherein the metallic matrix material comprises one or more of the following: a magnesium-based alloy; an aluminum-based alloy; or a zinc-based alloy.

## Embodiment 16

The method of any one of Embodiments 1 to 15, wherein the mixture comprises about 0.001 wt. % to about 10 wt. % of the disintegration agent, based on the total weight of the mixture.

## Embodiment 17

A degradable article produced by the method of any one of Embodiments 1 to 16.

## Embodiment 18

A degradable article comprising:  
a metallic matrix comprising a plurality of grains formed from a metallic matrix material, a carrier, or a combination thereof; and  
a disintegration agent disposed on grain boundaries of the grains formed from the metallic matrix material, the carrier, or a combination thereof; the disintegration agent comprising particles having an aspect ratio greater than about 2;

wherein the metallic matrix and the disintegration agent form a plurality of galvanic cells in the article.

Embodiment 19

The degradable article of Embodiment 18, wherein the disintegration agent comprises particles having an aspect ratio greater than about 5.

Embodiment 20

The degradable article of Embodiment 18 or Embodiment 19, wherein the disintegration agent is further disposed inside the grains formed from the metallic matrix material.

The use of the terms "a" and "an" and "the" and similar referents in the context of describing the invention (especially in the context of the following claims) are to be construed to cover both the singular and the plural, unless otherwise indicated herein or clearly contradicted by context. "Or" means "and/or." The modifier "about" used in connection with a quantity is inclusive of the stated value and has the meaning dictated by the context (e.g., it includes the degree of error associated with measurement of the particular quantity). As used herein, the size or average size of the particles refers to the largest dimension of the particles and can be determined by high resolution electron or atomic force microscope technology.

All references cited herein are incorporated by reference in their entirety. While typical embodiments have been set forth for the purpose of illustration, the foregoing descriptions should not be deemed to be a limitation on the scope herein. Accordingly, various modifications, adaptations, and alternatives can occur to one skilled in the art without departing from the spirit and scope herein.

What is claimed is:

1. A method of manufacturing a degradable article, the method comprising:
  - forming a mixture comprising composite particles dispersed in a metallic matrix material; the composite particles comprising a carrier and a disintegration agent coated on the carrier or embedded in the carrier, or a combination thereof and the composite particles having a density that is about 0.2 to about 2.5 equivalents to that of the metallic matrix material when measured under the same testing conditions;
  - releasing the disintegrating agent from the composite particles; and
  - molding or casting the mixture to form a degradable article;

wherein the disintegration agent forms a plurality of galvanic cells with the metallic matrix material, with the carrier, or with a combination of the metallic matrix material and the carrier, in the degradable article.
2. The method of claim 1 wherein the composite particles have a density that is about 0.5 to about 1.5 equivalents to that of the metallic matrix material when measured under the same testing conditions.
3. The method of claim 1, further comprising forming the composite particles by one or more of the following: physical vapor deposition; chemical vapor deposition; milling; or mechanical mixing.
4. The method of claim 1, wherein forming a mixture comprising composite particles dispersed in a metallic matrix material comprises:
  - mixing the metallic matrix material in a solid form with the composite particles to provide a blend; and

heating the blend to a temperature to selectively melt the metallic matrix material.

5. The method of claim 4, wherein the carrier is at least partially melted at the temperature.
6. The method of claim 1, wherein forming a mixture comprising composite particles dispersed in a metallic matrix material comprises:
  - heating the metallic matrix material in a solid form to provide a molten metallic matrix material; and
  - introducing the composite particles to the molten matrix material.
7. The method of claim 6, wherein heating the metallic matrix material is to a temperature of about 450° C. to about 850° C.
8. The method of claim 1, wherein molding the mixture comprises pressure molding or vacuum molding.
9. The method of claim 1, wherein molding the mixture comprises applying a superatmospheric pressure of about 500 psi to about 30,000 psi to the mixture.
10. The method of claim 1, further comprising extruding the molded article.
11. The method of claim 1, wherein the carrier comprises one or more of the following: a magnesium-based alloy; an aluminum-based alloy; or a zinc-based alloy.
12. The method of claim 1, wherein the carrier comprises particles have an average particle size of about 1 micron to about 10 millimeters.
13. The method of claim 1, wherein the disintegration agent comprises one or more of the following: a metal; an oxide of the metal; a nitride of the metal; or a cermet of the metal; wherein the metal is one or more of the following: W; Co; Cu; Ni; or Fe.
14. The method of claim 1, wherein the disintegration agent comprises particles having an average particle size of about 200 nanometers to about 10 microns.
15. The method of claim 1, wherein the metallic matrix material comprises one or more of the following: a magnesium-based alloy; an aluminum-based alloy; or a zinc-based alloy.
16. The method of claim 1, wherein the mixture comprises about 0.001 wt. % to about 10 wt. % of the disintegration agent, based on the total weight of the mixture.
17. A degradable article produced by the method of claim 1.
18. A degradable article comprising:
  - a metallic matrix comprising a plurality of grains formed from a metallic matrix material, a carrier, or a combination thereof; and
  - a disintegration agent disposed on grain boundaries of the grains formed from the metallic matrix material, the carrier, or a combination thereof; the disintegration agent comprising particles having an aspect ratio greater than about 2;

wherein the metallic matrix and the disintegration agent form a plurality of galvanic cells in the article; and the disintegration agent comprises one or more of the following: a metal; an oxide of the metal; a nitride of the metal; or a cermet of the metal; wherein the metal is one or more of the following: W; Co; Cu; Ni; or Fe.
19. The degradable article of claim 18, wherein the disintegration agent comprises particles having an aspect ratio greater than about 5.
20. The degradable article of claim 18, wherein the disintegration agent is further disposed inside the grains formed from the metallic matrix material.

**21.** The method of claim 1, wherein releasing the disintegration agent comprises partially or completely melting the carrier.

**22.** The method of claim 1, wherein the composite particles comprise the carrier and the disintegration agent 5 coated on the carrier.

**23.** The method of claim 1, wherein the composite particles comprise the carrier and the disintegration agent embedded in the carrier.

**24.** The method of claim 1, further comprising selectively 10 melting the matrix material and the carrier but not the disintegration agent.

\* \* \* \* \*